



US008864944B2

(12) **United States Patent**  
**Miller et al.**

(10) **Patent No.:** **US 8,864,944 B2**  
(45) **Date of Patent:** **\*Oct. 21, 2014**

(54) **METHOD OF MAKING A WIPER/TOWEL PRODUCT WITH CELLULOSIC MICROFIBERS**

(71) Applicant: **Georgia-Pacific Consumer Products LP**, Atlanta, GA (US)

(72) Inventors: **Joseph H. Miller**, Neenah, WI (US); **Daniel W. Sumnicht**, Hobart, WI (US); **Ayanna M. Bernard**, Neenah, WI (US); **Sanjay Wahal**, Appleton, WI (US)

(73) Assignee: **Georgia-Pacific Consumer Products LP**, Atlanta, GA (US)

(\*) Notice: Subject to any disclaimer, the term of this patent is extended or adjusted under 35 U.S.C. 154(b) by 0 days.

This patent is subject to a terminal disclaimer.

(21) Appl. No.: **13/942,835**

(22) Filed: **Jul. 16, 2013**

(65) **Prior Publication Data**

US 2013/0299105 A1 Nov. 14, 2013

**Related U.S. Application Data**

(63) Continuation of application No. 13/137,216, filed on Jul. 28, 2011, now Pat. No. 8,540,846, which is a continuation-in-part of application No. 12/694,650, filed on Jan. 27, 2010, now Pat. No. 8,293,072.

(60) Provisional application No. 61/206,146, filed on Jan. 28, 2009.

(51) **Int. Cl.**

**B31F 1/16** (2006.01)  
**D21H 27/40** (2006.01)  
**D21H 27/00** (2006.01)  
**B31F 1/12** (2006.01)  
**D21H 21/14** (2006.01)  
**D21H 11/18** (2006.01)  
**D21H 27/30** (2006.01)  
**D21H 25/00** (2006.01)  
**D21H 27/02** (2006.01)  
**D21F 11/00** (2006.01)

(52) **U.S. Cl.**

CPC ..... **D21H 27/007** (2013.01); **D21H 27/002** (2013.01); **B31F 1/126** (2013.01); **D21H 21/146** (2013.01); **D21H 11/18** (2013.01); **D21H 1/02** (2013.01); **B31F 1/16** (2013.01); **D21H 25/005** (2013.01); **D21H 27/02** (2013.01); **D21H 27/30** (2013.01); **D21F 11/006** (2013.01)

USPC ..... **162/111**; 162/117; 162/123; 162/146; 162/149; 162/157.6

(58) **Field of Classification Search**

CPC .... D21H 27/002; D21H 27/30; D21H 13/08; D21H 11/18; D21H 11/20; D21H 1/02; D21H 27/02; D21H 11/16; D21F 11/006; B31F 1/126; B31F 1/16

USPC ..... 162/9, 28, 109, 111, 117, 123–130, 162/141, 146, 149–150, 157.1, 157.6, 162/157.7, 182; 428/359, 391, 393, 304.4, 428/311.11, 311.51, 311.71, 156, 172; 264/282–284; 156/183

See application file for complete search history.

(56)

**References Cited**

U.S. PATENT DOCUMENTS

|             |         |                |
|-------------|---------|----------------|
| 1,983,529 A | 12/1934 | Brandenberger  |
| 2,025,000 A | 12/1935 | Losee          |
| 2,428,046 A | 9/1947  | Sisson et al.  |
| 2,440,761 A | 5/1948  | Sisson et al.  |
| 2,459,927 A | 1/1949  | Dreyfus et al. |
| 2,517,764 A | 8/1950  | Carson         |

(Continued)

FOREIGN PATENT DOCUMENTS

|                 |         |
|-----------------|---------|
| CA 1 002 359 A1 | 12/1976 |
| CA 2 053 505    | 4/1992  |

(Continued)

OTHER PUBLICATIONS

Miller, Bernard and Ilya Tyomkin. "Liquid Porosimetry: New Methodology and Applications," Journal of Colloid and Interface Science, 1994, 162, pp. 163–170, TRI/Princeton.

(Continued)

*Primary Examiner* — Jose Fortuna

(74) *Attorney, Agent, or Firm* — Laura L. Bozek

(57)

**ABSTRACT**

A method of making a multi-ply wiper/towel product with cellulosic microfibers. The method includes compactively dewatering a nascent web that includes at least about 10% fibrillated cellulosic microfibers and has an apparently random distribution of fibers. The dewatered web having the apparently random distribution of fibers is applied to a transfer surface. The web is belt-creped from the transfer surface utilizing a creping belt. The belt-creping step occurs under pressure in a belt creping nip defined between the transfer surface and the creping belt. The web is dried to form a dried web having a plurality of fiber-enriched hollow domed regions protruding from an upper side of the dried web. The hollow domed regions have a sidewall of a relatively high local basis weight formed along at least a leading edge thereof. The web also has connecting regions of a relatively lower local basis weight forming a network interconnecting the hollow domed regions of the dried web, and transition areas provided with upwardly and inwardly inflected consolidated fibrous regions that transition from the connecting regions into the sidewalls of the hollow domed regions formed along at least the leading edge thereof.

| (56)                  | References Cited |                        |             |         |                        |  |
|-----------------------|------------------|------------------------|-------------|---------|------------------------|--|
| U.S. PATENT DOCUMENTS |                  |                        |             |         |                        |  |
| 2,744,292 A           | 5/1956           | Schlosser et al.       | 4,849,054 A | 7/1989  | Klowak                 |  |
| 2,785,995 A           | 3/1957           | Kress                  | 4,906,513 A | 3/1990  | Kebbell et al.         |  |
| 3,009,822 A           | 11/1961          | Drelich et al.         | 4,908,097 A | 3/1990  | Box                    |  |
| 3,173,830 A           | 3/1965           | Wise et al.            | 4,931,201 A | 6/1990  | Julemont               |  |
| 3,175,339 A           | 3/1965           | McDowell               | 4,942,077 A | 7/1990  | Wendt et al.           |  |
| 3,209,402 A           | 10/1965          | Riley et al.           | 4,973,512 A | 11/1990 | Stanley et al.         |  |
| 3,337,671 A           | 8/1967           | Drisch et al.          | 4,987,632 A | 1/1991  | Rowe et al.            |  |
| 3,382,140 A           | 5/1968           | Henderson et al.       | 4,998,568 A | 3/1991  | Vohringer              |  |
| 3,432,936 A           | 3/1969           | Cole et al.            | 5,016,678 A | 5/1991  | Borel et al.           |  |
| 3,475,270 A           | 10/1969          | Cruz                   | 5,023,132 A | 6/1991  | Stanley et al.         |  |
| 3,508,941 A           | 4/1970           | Johnson                | 5,039,431 A | 8/1991  | Johnson et al.         |  |
| 3,692,622 A           | 9/1972           | Dunning                | 5,048,589 A | 9/1991  | Cook et al.            |  |
| 3,785,918 A           | 1/1974           | Kawai et al.           | 5,054,525 A | 10/1991 | Vohringer              |  |
| 3,926,716 A           | 12/1975          | Bates                  | 5,066,532 A | 11/1991 | Gaisser                |  |
| 3,974,025 A           | 8/1976           | Ayers                  | 5,087,324 A | 2/1992  | Awofeso et al.         |  |
| 3,994,771 A           | 11/1976          | Morgan, Jr. et al.     | 5,098,519 A | 3/1992  | Ramasubramanian et al. |  |
| 4,036,679 A           | 7/1977           | Back et al.            | 5,098,522 A | 3/1992  | Smurkoski et al.       |  |
| 4,064,213 A           | 12/1977          | Lazorisak et al.       | 5,103,874 A | 4/1992  | Lee                    |  |
| 4,100,324 A           | 7/1978           | Anderson et al.        | 5,114,777 A | 5/1992  | Gaisser                |  |
| 4,102,737 A           | 7/1978           | Morton                 | 5,124,197 A | 6/1992  | Bernardin et al.       |  |
| 4,125,659 A           | 11/1978          | Klowak et al.          | 5,129,988 A | 7/1992  | Farrington, Jr.        |  |
| 4,145,532 A           | 3/1979           | Franks et al.          | 5,137,600 A | 8/1992  | Barnes et al.          |  |
| 4,161,195 A           | 7/1979           | Khan                   | 5,167,261 A | 12/1992 | Lee                    |  |
| 4,182,381 A           | 1/1980           | Gisbourne              | 5,182,164 A | 1/1993  | Eklund et al.          |  |
| 4,184,519 A           | 1/1980           | McDonald et al.        | 5,199,467 A | 4/1993  | Lee                    |  |
| 4,196,282 A           | 4/1980           | Franks et al.          | 5,211,815 A | 5/1993  | Ramasubramanian et al. |  |
| 4,225,382 A           | 9/1980           | Kearney et al.         | 5,219,004 A | 6/1993  | Chiu                   |  |
| 4,239,065 A           | 12/1980          | Trokhman               | 5,223,096 A | 6/1993  | Phan et al.            |  |
| 4,246,221 A           | 1/1981           | McCorsley, III         | 5,225,269 A | 7/1993  | Bohlin                 |  |
| 4,307,143 A           | 12/1981          | Meitner                | 5,227,024 A | 7/1993  | Gomez                  |  |
| 4,314,589 A           | 2/1982           | Buchanan et al.        | 5,245,025 A | 9/1993  | Trokhman et al.        |  |
| 4,356,059 A           | 10/1982          | Hostettler             | 5,269,470 A | 12/1993 | Ishikawa et al.        |  |
| 4,359,069 A           | 11/1982          | Hahn                   | 5,277,761 A | 1/1994  | Van Phan et al.        |  |
| 4,374,702 A           | 2/1983           | Turbak et al.          | 5,314,584 A | 5/1994  | Grinnell et al.        |  |
| 4,376,455 A           | 3/1983           | Hahn                   | 5,320,710 A | 6/1994  | Reeves et al.          |  |
| 4,379,735 A           | 4/1983           | MacBean                | 5,328,565 A | 7/1994  | Rasch et al.           |  |
| 4,420,372 A           | 12/1983          | Hostettler             | 5,336,373 A | 8/1994  | Scattolino et al.      |  |
| 4,426,228 A           | 1/1984           | Brandner et al.        | 5,348,620 A | 9/1994  | Hermans et al.         |  |
| 4,426,417 A           | 1/1984           | Meitner et al.         | 5,354,524 A | 10/1994 | Sellars et al.         |  |
| 4,436,780 A           | 3/1984           | Hotchkiss et al.       | 5,366,785 A | 11/1994 | Sawdai                 |  |
| 4,440,597 A           | 4/1984           | Wells et al.           | 5,368,696 A | 11/1994 | Cunnane, III et al.    |  |
| 4,441,962 A           | 4/1984           | Osborn, III            | 5,372,876 A | 12/1994 | Johnson et al.         |  |
| 4,448,638 A           | 5/1984           | Klowak                 | 5,379,808 A | 1/1995  | Chiu                   |  |
| 4,453,573 A           | 6/1984           | Thompson               | 5,385,640 A | 1/1995  | Weibel et al.          |  |
| 4,468,428 A           | 8/1984           | Early et al.           | 5,411,636 A | 5/1995  | Hermans et al.         |  |
| 4,481,076 A           | 11/1984          | Herrick                | 5,451,353 A | 9/1995  | Rezai et al.           |  |
| 4,481,077 A           | 11/1984          | Herrick                | 5,492,598 A | 2/1996  | Hermans et al.         |  |
| 4,482,429 A           | 11/1984          | Klowak                 | 5,494,554 A | 2/1996  | Edwards et al.         |  |
| 4,483,743 A           | 11/1984          | Turbak et al.          | 5,501,768 A | 3/1996  | Hermans et al.         |  |
| 4,490,925 A           | 1/1985           | Smith                  | 5,503,715 A | 4/1996  | Trokhman et al.        |  |
| 4,507,173 A           | 3/1985           | Klowak et al.          | 5,505,818 A | 4/1996  | Hermans et al.         |  |
| 4,528,239 A           | 7/1985           | Trokhman               | 5,510,001 A | 4/1996  | Hermans et al.         |  |
| 4,528,316 A           | 7/1985           | Sorens                 | 5,510,002 A | 4/1996  | Hermans et al.         |  |
| 4,529,480 A           | 7/1985           | Trokhman               | 5,549,790 A | 8/1996  | Van Phan               |  |
| 4,533,437 A           | 8/1985           | Curran et al.          | 5,556,509 A | 9/1996  | Trokhman et al.        |  |
| 4,543,156 A           | 9/1985           | Cheshire et al.        | 5,562,739 A | 10/1996 | Urben                  |  |
| 4,546,052 A           | 10/1985          | Nicoll                 | 5,580,356 A | 12/1996 | Taylor                 |  |
| 4,551,199 A           | 11/1985          | Weldon                 | 5,582,681 A | 12/1996 | Back et al.            |  |
| 4,552,709 A           | 11/1985          | Koger, II et al.       | 5,593,545 A | 1/1997  | Rugowski et al.        |  |
| 4,556,450 A           | 12/1985          | Chuang et al.          | 5,601,871 A | 2/1997  | Krzysik et al.         |  |
| 4,592,395 A           | 6/1986           | Borel                  | 5,607,551 A | 3/1997  | Farrington, Jr. et al. |  |
| 4,605,585 A           | 8/1986           | Johansson              | 5,609,725 A | 3/1997  | Van Phan               |  |
| 4,610,743 A           | 9/1986           | Salmeen et al.         | 5,614,293 A | 3/1997  | Krzysik et al.         |  |
| 4,611,639 A           | 9/1986           | Bugge                  | 5,618,612 A | 4/1997  | Gstrein                |  |
| 4,614,679 A           | 9/1986           | Farrington, Jr. et al. | H001672 H   | 8/1997  | Hermans et al.         |  |
| 4,637,859 A           | 1/1987           | Trokhman               | 5,656,132 A | 8/1997  | Farrington, Jr. et al. |  |
| 4,640,741 A           | 2/1987           | Tsuneo                 | 5,657,797 A | 8/1997  | Townley et al.         |  |
| 4,689,119 A           | 8/1987           | Weldon                 | 5,667,636 A | 9/1997  | Engel et al.           |  |
| 4,709,732 A           | 12/1987          | Kinnunen               | 5,672,248 A | 9/1997  | Wendt et al.           |  |
| 4,735,849 A           | 4/1988           | Murakami et al.        | 5,674,590 A | 10/1997 | Anderson et al.        |  |
| 4,759,391 A           | 7/1988           | Waldvogel et al.       | 5,688,468 A | 11/1997 | Lu                     |  |
| 4,759,976 A           | 7/1988           | Dutt                   | 5,690,149 A | 11/1997 | Lee                    |  |
| 4,795,530 A           | 1/1989           | Soerens et al.         | 5,695,607 A | 12/1997 | Oriaran et al.         |  |
| 4,802,942 A           | 2/1989           | Takemura et al.        | 5,725,734 A | 3/1998  | Herman et al.          |  |
| 4,834,838 A           | 5/1989           | Klowak                 | 5,725,821 A | 3/1998  | Gannon et al.          |  |
|                       |                  |                        | 5,746,887 A | 5/1998  | Wendt et al.           |  |
|                       |                  |                        | 5,759,210 A | 6/1998  | Potter et al.          |  |
|                       |                  |                        | 5,759,926 A | 6/1998  | Pike et al.            |  |
|                       |                  |                        | 5,772,845 A | 6/1998  | Farrington, Jr. et al. |  |

| (56) References Cited |         |                        |              |         |                   |
|-----------------------|---------|------------------------|--------------|---------|-------------------|
| U.S. PATENT DOCUMENTS |         |                        |              |         |                   |
| 5,779,737 A           | 7/1998  | Potter et al.          | 6,514,613 B2 | 2/2003  | Luo et al.        |
| 5,814,190 A           | 9/1998  | Van Phan               | 6,533,898 B2 | 3/2003  | Gross             |
| 5,830,321 A           | 11/1998 | Lindsay et al.         | 6,534,151 B2 | 3/2003  | Merker            |
| 5,840,403 A           | 11/1998 | Trokhann et al.        | 6,540,879 B2 | 4/2003  | Marinack et al.   |
| 5,840,404 A           | 11/1998 | Graff                  | 6,544,912 B1 | 4/2003  | Tanio et al.      |
| 5,851,353 A           | 12/1998 | Fiscus et al.          | 6,547,924 B2 | 4/2003  | Klerelid et al.   |
| 5,858,021 A           | 1/1999  | Sun et al.             | 6,551,461 B2 | 4/2003  | Leitner et al.    |
| 5,863,652 A           | 1/1999  | Matsumura et al.       | 6,558,511 B2 | 5/2003  | Dwiggins et al.   |
| 5,865,955 A           | 2/1999  | Ilvespaa et al.        | 6,565,707 B2 | 5/2003  | Behnke et al.     |
| 5,866,407 A           | 2/1999  | Foody et al.           | 6,573,204 B1 | 6/2003  | Philipp et al.    |
| 5,888,347 A           | 3/1999  | Engel et al.           | 6,585,855 B2 | 7/2003  | Drew et al.       |
| 5,895,710 A           | 4/1999  | Sasse et al.           | 6,596,033 B1 | 7/2003  | Luo et al.        |
| 5,932,068 A           | 8/1999  | Farrington, Jr. et al. | 6,602,386 B1 | 8/2003  | Takeuchi et al.   |
| 5,935,381 A           | 8/1999  | Trokhann et al.        | 6,607,638 B2 | 8/2003  | Drew et al.       |
| 5,935,681 A           | 8/1999  | Paulett                | 6,610,173 B1 | 8/2003  | Lindsay et al.    |
| 5,935,880 A           | 8/1999  | Wang et al.            | 6,624,100 B1 | 9/2003  | Pike              |
| 5,958,187 A           | 9/1999  | Bhat et al.            | 6,645,420 B1 | 11/2003 | Beck              |
| 5,964,983 A           | 10/1999 | Dinand et al.          | 6,645,618 B2 | 11/2003 | Hobbs et al.      |
| 5,968,590 A           | 10/1999 | Ahonen et al.          | 6,660,362 B1 | 12/2003 | Lin et al.        |
| 6,001,218 A           | 12/1999 | Hsu et al.             | 6,669,821 B2 | 12/2003 | Edwards et al.    |
| 6,001,421 A           | 12/1999 | Ahonen et al.          | 6,692,827 B2 | 2/2004  | Luo et al.        |
| 6,017,417 A           | 1/2000  | Wendt et al.           | 6,699,806 B1 | 3/2004  | Marinack et al.   |
| 6,027,611 A           | 2/2000  | McFarland et al.       | 6,746,558 B2 | 6/2004  | Hoeft et al.      |
| 6,033,523 A           | 3/2000  | Dwiggins et al.        | 6,746,976 B1 | 6/2004  | Urankar et al.    |
| 6,036,820 A           | 3/2000  | Schiel et al.          | 6,749,718 B2 | 6/2004  | Takai et al.      |
| 6,042,769 A           | 3/2000  | Gannon et al.          | 6,752,907 B2 | 6/2004  | Edwards et al.    |
| 6,048,641 A           | 4/2000  | Ohmory et al.          | 6,767,634 B2 | 7/2004  | Krishnaswamy      |
| 6,059,928 A           | 5/2000  | Van Luu et al.         | 6,773,648 B2 | 8/2004  | Luo et al.        |
| 6,080,279 A           | 6/2000  | Hada et al.            | 6,797,115 B2 | 9/2004  | Klerelid et al.   |
| 6,083,346 A           | 7/2000  | Hermans et al.         | 6,808,557 B2 | 10/2004 | Holbrey et al.    |
| 6,093,284 A           | 7/2000  | Hada et al.            | 6,824,599 B2 | 11/2004 | Swatoski et al.   |
| 6,096,169 A           | 8/2000  | Hermans et al.         | 6,824,648 B2 | 11/2004 | Edwards et al.    |
| 6,117,525 A           | 9/2000  | Trokhann et al.        | 6,827,819 B2 | 12/2004 | Dwiggins et al.   |
| 6,117,545 A           | 9/2000  | Cavaille et al.        | 6,833,187 B2 | 12/2004 | Luo et al.        |
| 6,119,362 A           | 9/2000  | Sundqvist              | 6,835,311 B2 | 12/2004 | Koslow            |
| 6,136,146 A           | 10/2000 | Phan et al.            | 6,841,038 B2 | 1/2005  | Horenziak et al.  |
| 6,139,686 A           | 10/2000 | Trokhann et al.        | 6,849,239 B2 | 2/2005  | Morris            |
| 6,143,135 A           | 11/2000 | Hada et al.            | 6,861,023 B2 | 3/2005  | Sealey, II et al. |
| 6,146,499 A           | 11/2000 | Lin et al.             | 6,872,311 B2 | 3/2005  | Koslow            |
| 6,149,767 A           | 11/2000 | Hermans et al.         | 6,890,649 B2 | 5/2005  | Hobbs et al.      |
| 6,153,136 A           | 11/2000 | Collier et al.         | 6,899,790 B2 | 5/2005  | Lee               |
| 6,162,327 A           | 12/2000 | Batra et al.           | 6,951,895 B1 | 10/2005 | Qin et al.        |
| 6,171,442 B1          | 1/2001  | Farrington, Jr. et al. | 6,964,117 B2 | 11/2005 | Parent            |
| 6,183,596 B1          | 2/2001  | Matsuda et al.         | 6,969,443 B1 | 11/2005 | Kokko             |
| 6,187,137 B1          | 2/2001  | Druecke et al.         | 6,986,932 B2 | 1/2006  | Zink et al.       |
| 6,197,154 B1          | 3/2001  | Chen et al.            | 6,998,017 B2 | 2/2006  | Lindsay et al.    |
| 6,210,528 B1          | 4/2001  | Wolkowicz              | 6,998,022 B2 | 2/2006  | Hultcrantz        |
| 6,214,163 B1          | 4/2001  | Matsuda et al.         | 7,037,405 B2 | 5/2006  | Nguyen et al.     |
| 6,221,487 B1          | 4/2001  | Luo et al.             | 7,067,444 B2 | 6/2006  | Luo et al.        |
| 6,315,864 B2          | 11/2001 | Anderson et al.        | 7,070,678 B2 | 7/2006  | Allen et al.      |
| 6,318,727 B1          | 11/2001 | Hada                   | 7,083,704 B2 | 8/2006  | Sealey, II et al. |
| 6,331,230 B1          | 12/2001 | Hermans et al.         | 7,094,317 B2 | 8/2006  | Lundberg et al.   |
| 6,350,349 B1          | 2/2002  | Hermans et al.         | 7,097,737 B2 | 8/2006  | Luo et al.        |
| 6,379,496 B2          | 4/2002  | Edwards et al.         | 7,160,418 B2 | 1/2007  | Edwards et al.    |
| 6,381,868 B1          | 5/2002  | Grabscheid et al.      | 7,195,694 B2 | 3/2007  | Von Drach et al.  |
| 6,413,368 B1          | 7/2002  | Dwiggins et al.        | 7,210,205 B2 | 5/2007  | Takeuchi et al.   |
| 6,416,631 B1          | 7/2002  | Beck                   | 7,214,633 B2 | 5/2007  | Sun et al.        |
| 6,419,793 B1          | 7/2002  | Beck                   | 7,229,528 B2 | 6/2007  | Vinson et al.     |
| 6,420,013 B1          | 7/2002  | Vinson et al.          | 7,241,711 B2 | 7/2007  | Takai et al.      |
| 6,432,267 B1          | 8/2002  | Watson                 | 7,250,382 B2 | 7/2007  | Takai et al.      |
| 6,432,270 B1          | 8/2002  | Liu et al.             | 7,258,764 B2 | 8/2007  | Mauler            |
| 6,436,234 B1          | 8/2002  | Chen et al.            | 7,276,166 B2 | 10/2007 | Koslow            |
| 6,440,547 B1          | 8/2002  | Luo et al.             | 7,276,459 B1 | 10/2007 | Lang et al.       |
| 6,444,314 B1          | 9/2002  | Luo et al.             | 7,296,691 B2 | 11/2007 | Koslow            |
| 6,447,640 B1          | 9/2002  | Watson et al.          | 7,300,543 B2 | 11/2007 | Mullally et al.   |
| 6,447,641 B1          | 9/2002  | Wolkowicz et al.       | 7,320,743 B2 | 1/2008  | Freidbauer et al. |
| 6,454,904 B1          | 9/2002  | Hermans et al.         | 7,381,294 B2 | 6/2008  | Suzuki et al.     |
| 6,461,474 B1          | 10/2002 | Lindsay et al.         | 7,387,706 B2 | 6/2008  | Herman et al.     |
| 6,464,829 B1          | 10/2002 | Chen et al.            | 7,399,378 B2 | 7/2008  | Edwards et al.    |
| 6,471,727 B2          | 10/2002 | Luo et al.             | 7,416,637 B2 | 8/2008  | Murray et al.     |
| 6,478,927 B1          | 11/2002 | Chen et al.            | 7,435,312 B2 | 10/2008 | Lindsay et al.    |
| 6,491,788 B2          | 12/2002 | Sealey, II et al.      | 7,442,278 B2 | 10/2008 | Murray et al.     |
| 6,497,789 B1          | 12/2002 | Hermans et al.         | 7,494,563 B2 | 2/2009  | Edwards et al.    |
| 6,500,302 B2          | 12/2002 | Dwiggins et al.        | 7,503,998 B2 | 3/2009  | Murray et al.     |
| 6,511,746 B1          | 1/2003  | Collier et al.         | 7,563,344 B2 | 7/2009  | Beuther et al.    |

(56)

## References Cited

## U.S. PATENT DOCUMENTS

|                 |         |                            |                 |         |                   |
|-----------------|---------|----------------------------|-----------------|---------|-------------------|
| 7,566,014 B2    | 7/2009  | Koslow et al.              | 2003/0203695 A1 | 10/2003 | Polanco et al.    |
| 7,585,388 B2    | 9/2009  | Yeh et al.                 | 2004/0038031 A1 | 2/2004  | Holbrey et al.    |
| 7,585,389 B2    | 9/2009  | Yeh et al.                 | 2004/0103507 A1 | 6/2004  | Takeuchi et al.   |
| 7,585,392 B2    | 9/2009  | Kokko et al.               | 2004/0203306 A1 | 10/2004 | Grafe et al.      |
| 7,588,660 B2    | 9/2009  | Edwards et al.             | 2004/0207110 A1 | 10/2004 | Luo et al.        |
| 7,588,661 B2    | 9/2009  | Edwards et al.             | 2004/0238135 A1 | 12/2004 | Edwards et al.    |
| 7,588,831 B2    | 9/2009  | Akiyama et al.             | 2004/0248494 A1 | 12/2004 | Hartgrove et al.  |
| 7,605,096 B2    | 10/2009 | Tomarchio et al.           | 2004/0256066 A1 | 12/2004 | Lindsay et al.    |
| 7,608,164 B2    | 10/2009 | Chou et al.                | 2005/0074542 A1 | 4/2005  | Lundberg et al.   |
| 7,651,589 B2    | 1/2010  | Murray et al.              | 2005/0136772 A1 | 6/2005  | Chen et al.       |
| 7,655,112 B2    | 2/2010  | Koslow                     | 2005/0148264 A1 | 7/2005  | Varona et al.     |
| 7,662,255 B2    | 2/2010  | Murray et al.              | 2005/0176326 A1 | 8/2005  | Bond et al.       |
| 7,662,257 B2    | 2/2010  | Edwards et al.             | 2005/0268274 A1 | 12/2005 | Beuther et al.    |
| 7,670,457 B2    | 3/2010  | Murray et al.              | 2005/0274469 A1 | 12/2005 | Lundberg et al.   |
| 7,691,228 B2    | 4/2010  | Edwards et al.             | 2005/0288484 A1 | 12/2005 | Holbrey et al.    |
| 7,691,760 B2    | 4/2010  | Bergsten et al.            | 2006/0088696 A1 | 4/2006  | Manifold et al.   |
| 7,700,764 B2    | 4/2010  | Heijnesson-Hulten          | 2006/0090271 A1 | 5/2006  | Price et al.      |
| 7,704,349 B2    | 4/2010  | Edwards et al.             | 2006/0141881 A1 | 6/2006  | Bergsten et al.   |
| 7,718,036 B2    | 5/2010  | Sumnicht et al.            | 2006/0207722 A1 | 9/2006  | Amano et al.      |
| 7,726,349 B2    | 6/2010  | Mullally et al.            | 2006/0240727 A1 | 10/2006 | Price et al.      |
| 7,744,723 B2    | 6/2010  | Sheehan et al.             | 2006/0240728 A1 | 10/2006 | Price et al.      |
| 7,758,723 B2    | 7/2010  | Vinson et al.              | 2006/0241287 A1 | 10/2006 | Hecht et al.      |
| 7,763,715 B2    | 7/2010  | Hecht et al.               | 2007/0062656 A1 | 3/2007  | Murray et al.     |
| 7,785,443 B2    | 8/2010  | Hermans et al.             | 2007/0137807 A1 | 6/2007  | Schulz et al.     |
| 7,789,995 B2    | 9/2010  | Super et al.               | 2007/0137814 A1 | 6/2007  | Gao               |
| 7,794,566 B2    | 9/2010  | Edwards et al.             | 2007/0224419 A1 | 9/2007  | Sumnicht et al.   |
| 7,799,968 B2    | 9/2010  | Chen et al.                | 2007/0228064 A1 | 10/2007 | Brennan et al.    |
| 7,811,418 B2    | 10/2010 | Klerlid et al.             | 2007/0232180 A1 | 10/2007 | Polat et al.      |
| 7,820,008 B2    | 10/2010 | Edwards et al.             | 2008/0008865 A1 | 1/2008  | Luu et al.        |
| 7,828,931 B2    | 11/2010 | Edwards et al.             | 2008/0029235 A1 | 2/2008  | Edwards et al.    |
| 7,850,823 B2    | 12/2010 | Chou et al.                | 2008/0057307 A1 | 3/2008  | Koslow et al.     |
| 7,871,493 B2    | 1/2011  | Hermans et al.             | 2008/0076313 A1 | 3/2008  | Uitenbroek et al. |
| 7,884,037 B2    | 2/2011  | Sirovatka et al.           | 2008/0145664 A1 | 6/2008  | Sirovatka et al.  |
| 7,888,412 B2    | 2/2011  | Holbrey et al.             | 2008/0173418 A1 | 7/2008  | Sumnicht          |
| 7,918,964 B2    | 4/2011  | Edwards et al.             | 2008/0173419 A1 | 7/2008  | Sumnicht          |
| 7,927,456 B2    | 4/2011  | Murray et al.              | 2008/0311815 A1 | 12/2008 | Gupta et al.      |
| 7,935,220 B2    | 5/2011  | Edwards et al.             | 2009/0020139 A1 | 1/2009  | Sumnicht et al.   |
| 7,951,264 B2    | 5/2011  | Sumnicht                   | 2009/0020248 A1 | 1/2009  | Sumnicht et al.   |
| 7,951,266 B2    | 5/2011  | Kokko et al.               | 2009/0120598 A1 | 5/2009  | Edwards et al.    |
| 7,972,474 B2    | 7/2011  | Underhill et al.           | 2009/0120599 A1 | 5/2009  | Nguyen            |
| 7,985,321 B2    | 7/2011  | Sumnicht et al.            | 2009/0126884 A1 | 5/2009  | Murray et al.     |
| 7,998,313 B2    | 8/2011  | Kokko                      | 2009/0151881 A1 | 6/2009  | Nguyen            |
| 8,012,312 B2    | 9/2011  | Goto et al.                | 2009/0159224 A1 | 6/2009  | Chou et al.       |
| 8,022,267 B2    | 9/2011  | Hellstrom et al.           | 2009/0259208 A1 | 10/2009 | Hellstrom et al.  |
| 8,030,231 B2    | 10/2011 | Lange et al.               | 2009/0308551 A1 | 12/2009 | Kokko et al.      |
| 8,066,849 B2    | 11/2011 | Kokko et al.               | 2010/0065235 A1 | 3/2010  | Fike et al.       |
| 8,105,463 B2    | 1/2012  | Goulet et al.              | 2010/0098191 A1 | 4/2010  | Hartgrove et al.  |
| 8,142,612 B2    | 3/2012  | Murray et al.              | 2010/0136268 A1 | 6/2010  | Rasch             |
| 8,152,957 B2    | 4/2012  | Edwards et al.             | 2010/0186913 A1 | 7/2010  | Super et al.      |
| 8,152,958 B2    | 4/2012  | Super et al.               | 2010/0212850 A1 | 8/2010  | Sumnicht et al.   |
| 8,177,938 B2    | 5/2012  | Sumnicht                   | 2010/0236735 A1 | 9/2010  | Goulet et al.     |
| 8,187,421 B2    | 5/2012  | Sumnicht et al.            | 2010/0272938 A1 | 10/2010 | Mitchell et al.   |
| 8,187,422 B2    | 5/2012  | Sumnicht et al.            | 2010/0282423 A1 | 11/2010 | Super et al.      |
| 8,216,425 B2    | 7/2012  | Sumnicht et al.            | 2010/0288456 A1 | 11/2010 | Westland et al.   |
| 8,226,797 B2    | 7/2012  | Murray et al.              | 2011/0011545 A1 | 1/2011  | Edwards et al.    |
| 8,257,552 B2    | 9/2012  | Edwards et al.             | 2011/0155337 A1 | 6/2011  | Murray et al.     |
| 8,293,072 B2    | 10/2012 | Super et al.               | 2011/0265965 A1 | 11/2011 | Sumnicht et al.   |
| 8,318,859 B2    | 11/2012 | Amano et al.               | 2011/0272304 A1 | 11/2011 | Wahal et al.      |
| 8,361,278 B2    | 1/2013  | Fike et al.                | 2012/0021178 A1 | 1/2012  | Miller et al.     |
| 8,410,005 B2    | 4/2013  | Brennan et al.             | 2012/0080155 A1 | 4/2012  | Konishi et al.    |
| 8,444,808 B2    | 5/2013  | Koslow et al.              | 2012/0180815 A1 | 7/2012  | Sumnicht et al.   |
| 8,513,147 B2    | 8/2013  | Gupta et al.               | 2012/0241113 A1 | 9/2012  | Super et al.      |
| 8,540,846 B2 *  | 9/2013  | Miller et al. .... 162/129 | 2013/0029105 A1 | 1/2013  | Miller et al.     |
| 2002/0162635 A1 | 11/2002 | Hsu et al.                 | 2013/0029106 A1 | 6/2013  | Miller et al.     |
| 2002/0168912 A1 | 11/2002 | Bond et al.                | 2013/0299106 A1 | 11/2013 | Miller et al.     |
| 2002/0187307 A1 | 12/2002 | Tanaka et al.              |                 |         |                   |
| 2003/0099821 A1 | 5/2003  | Takai et al.               | EP 0 279 465 A2 | 8/1988  |                   |
| 2003/0100240 A1 | 5/2003  | Takai et al.               | EP 0 399 522 A2 | 11/1990 |                   |
| 2003/0111195 A1 | 6/2003  | Hu                         | EP 0 485 360 A2 | 5/1992  |                   |
| 2003/0144640 A1 | 7/2003  | Nguyen                     | EP 1 036 880 A1 | 9/2000  |                   |
| 2003/0157351 A1 | 8/2003  | Swatloski et al.           | EP 1 302 146 A2 | 4/2003  |                   |
| 2003/0168401 A1 | 9/2003  | Koslow                     | GB 978953 A     | 1/1965  |                   |
| 2003/0177909 A1 | 9/2003  | Koslow                     | GB 2 319 537 A  | 5/1998  |                   |
| 2003/0178166 A1 | 9/2003  | Takeuchi et al.            | GB 2 412 083 A  | 9/2005  |                   |
| 2003/0200991 A1 | 10/2003 | Keck et al.                | JP 8003890 A    | 1/1996  |                   |
|                 |         |                            | RU 2127343 C1   | 3/1999  |                   |

## FOREIGN PATENT DOCUMENTS

(56)

## References Cited

## FOREIGN PATENT DOCUMENTS

RU 2143508 C1 12/1999  
 RU 2144101 C1 1/2000  
 RU 2183648 C2 6/2002  
 RU 2226231 C1 3/2004  
 RU 2328255 C2 7/2008  
 WO 95/35399 A1 12/1995  
 WO 96/06223 A1 2/1996  
 WO 97/43484 A1 11/1997  
 WO 98/03710 A1 1/1998  
 WO 98/07914 A1 2/1998  
 WO 00/14330 A1 3/2000  
 WO 00/36212 A1 6/2000  
 WO 00/40405 A1 7/2000  
 WO 02/02869 A2 1/2002  
 WO 02/40769 A2 5/2002  
 WO 2004/033793 A2 4/2004  
 WO 2005/010273 A1 2/2005  
 WO 2005/106117 A1 11/2005  
 WO 2006/113025 A2 10/2006  
 WO 2006/115817 A2 11/2006  
 WO 2007/001837 A2 1/2007  
 WO 2007/109259 A2 9/2007  
 WO 2007/139726 A1 12/2007  
 WO 2008/045770 A2 4/2008  
 WO 2008/146454 A1 12/2008  
 WO 2008/156454 A1 12/2008  
 WO 2009/038730 A1 3/2009  
 WO 2009/038735 A1 3/2009  
 WO 2010/088359 A1 8/2010  
 WO 2011/069532 A1 6/2011

## OTHER PUBLICATIONS

Gooding, R.W. and J.A. Olson. "Fractionation in a Bauer-McNett Classifier," *Journal of Pulp and Paper Science*, Dec. 12, 2001, vol. 27, No. 12, pp. 423-428.

Imperato, Giovanni, et al. "Low-melting sugar-urea-salt mixtures as solvents for Diels-Alder reactions," *Chemical Communications*, 2005, Issue 9, pp. 1170-1172, RSC Publishing.

Ozturk, Hale Bahar and Thomas Bechtold, "Splitting Tendency of Cellulosic Fibers," *Lenzinger Berichte*, 84, 2005, pp. 123-129.  
 Sung, Y.J., et al., "Applications of Thickness and Apparent Density Mapping by Laser Profilometry," 13th Fundamental Research Symposium, Cambridge, Sep. 2005, pp. 961-1007.  
 Klerlid, Ingvar and Ola Thomasson, "Advantage (TM) NTT (TM): low energy, high quality," *Tissue World*, Oct./Nov. 2008, pp. 49-52.  
 Dymrose-Peterson, Katherine. "Smart Materials for Liquid Control," *Nonwovens World*, Oct.-Nov. 1999, pp. 95-99.  
 Keller, D.S. and J.J. Pawlak, "B(Beta)-Radiographic Imaging of Paper Formation Using Storage Phosphor Screens," *Journal of Pulp and Paper Science*, vol. 27, No. 4, Apr. 2001, pp. 117-123.  
 Waterhouse, J.F. "On-Line Formation Measurements and Paper Quality," *Institute of Paper Science and Technology*, 1996, IPST Technical Paper Series 604.  
 Cresson, Thierry M., et al. "Characterization of paper formation Part 1: sensing paper formation," *Tappi Journal*, Jul. 1990, pp. 153-159.  
 International Search Report mailed Mar. 27, 2013, issued in corresponding International Application No. PCT/US2012/048046.  
 Written Opinion of the International Searching Authority mailed Mar. 27, 2013, issued in corresponding International Application No. PCT/US2012/048046.  
 International Search Report and Written Opinion of the International Searching Authority mailed Jul. 2, 2010, issued in corresponding International Application No. PCT/US2009/057078.  
 International Search Report and Written Opinion of the International Searching Authority mailed Jun. 4, 2010, issued in corresponding International Application No. PCT/US07/06892.  
 International Search Report and Written Opinion of the International Searching Authority mailed Dec. 1, 2008, issued in corresponding International Application No. PCT/US08/10840.  
 International Search Report and Written Opinion of the International Searching Authority mailed Dec. 12, 2008, issued in corresponding International Application No. PCT/US08/10833.  
 Notification of and International Preliminary Report on Patentability issued May 2, 2014, and mailed May 12, 2014, in counterpart International Application No. PCT/US12/48046.  
 Notification of and International Preliminary Report on Patentability completed Jan. 28, 2014, and mailed Feb. 6, 2014, in corresponding International Application No. PCT/US2012/048046.

\* cited by examiner

*FIG. 1A*

FRFC, 50% CMF

*FIG. 1B*

CELL 2, 0% CMF

*FIG. 1C*

FRFC, 50% CMF

*FIG. 1D*

CELL 2, 0% CMF

*FIG. 1E*



FRFC, 50% CMF

*FIG. 1F*



CELL 2, 0% CMF

*FIG. 1G*

FRBC, 40% CMF

*FIG. 1H*

TAD, 0% CMF

FIG. 1J



FIG. 1K



*FIG. 1L*



FRBC, 40% CMF

*FIG. 1M*



TAD, 0% CMF

*FIG. 1N*



CWP, 50% CMF

*FIG. 1P*



CWP, 0% CMF

*FIG. 10*



CWP, 50% CMF

*FIG. 1R*



CWP, 0% CMF

*FIG. 1S*



CWP, 50% CMF

*FIG. 1T*



CWP, 0% CMF

**FIG. 2**  
WIPE DRY TIMES FOR FRBC TWO-PLY WIPER



FIG. 3



FIG. 4



FIG. 5



*FIG. 6*



FIG. 7



FIG. 8



FIG. 9

## PORE VOLUME DISTRIBUTION SAMPLE CONFIGURATION



FIG. 10



FIG. 11



FIG. 12



FIG. 13



FIG. 14



FIG. 15



FIG. 16



FIG. 17



FIG. 18



FIG. 19



FIG. 20



FIG. 21



FIG. 22



FIG. 23

## VISCONIP PRESS ADJUSTMENTS FOR CMF



FIG. 24

EFFECT OF CMF ON BULK AT CONSTANT PRESSING



*FIG. 25A*



*FIG. 25B*



*FIG. 26*



BELT-CREPED WIPER EMBOSSED PATTERN

FIG. 27



FIG. 28



FIG. 28



FIG. 30



FIG. 31



FIG. 32



FIG. 39



SAT CAPACITY AND WIPE DRY TIME VERSUS CELL ID

*FIG. 34*  
18" Hg, VACUUM, UNCALENDERED, BELT 50, MD



**FIG. 35**

18" Hg VACUUM, UNCALENDERED, BELT 50, MD

660

662

610

600

658

618

620

NTE-EP

X128 16.5 μm

15kV



**FIG. 36**  
18" Hg VACUUM, CALENDERED, BELT 50, MD



FIG. 37



FIG. 38



FIG. 39



FIG. 40



FIG. 41



FIG. 42



**METHOD OF MAKING A WIPER/TOWEL  
PRODUCT WITH CELLULOSIC  
MICROFIBERS**

**CROSS-REFERENCE TO RELATED  
APPLICATIONS AND INCORPORATION BY  
REFERENCE**

This application is a continuation application of U.S. patent application Ser. No. 13/137,216, filed on Jul. 28, 2011, published on Jan. 26, 2012, as U.S. Patent Application Publication No. 2012/0021178, now U.S. Pat. No. 8,540,846, which is a continuation in part of U.S. patent application Ser. No. 12/694,650, filed Jan. 27, 2010, U.S. Patent Application Publication No. 2010/0186913, entitled "Belt-Creped, Variable Local Basis Weight Absorbent Sheet Prepared With Perforated Polymeric Belt", published Jul. 29, 2010, now U.S. Pat. No. 8,293,072, which was based upon U.S. Provisional Patent Application No. 61/206,146, filed Jan. 28, 2009, the right of priority of the foregoing being hereby claimed. All of the foregoing applications are incorporated herein by reference.

This application relates to the subject matter of U.S. Patent Application Publication No. 2009/0020139, published Jan. 22, 2009, based on U.S. patent application Ser. No. 12/284,148, filed Sep. 17, 2008, now U.S. Pat. No. 8,187,422, entitled "High Efficiency Disposable Cellulosic Wiper". This application also relates to the subject matter of U.S. Patent Application Publication No. 2009/0020248, published Jan. 22, 2009, based on U.S. patent application Ser. No. 12/284,147, also filed Sep. 17, 2008, now U.S. Pat. No. 8,187,421, entitled "Absorbent Sheet Incorporating Regenerated Cellulose Microfiber". Both U.S. patent application Ser. Nos. 12/284,148 and 12/284,147 were based, in part, on U.S. patent application Ser. No. 11/725,253, filed Mar. 19, 2007, entitled "Absorbent Sheet Having Regenerated Cellulose Microfiber Network", now U.S. Pat. No. 7,718,036. This application also relates, in part, to the subject matter of the following U.S. Provisional Patent Applications:

- (1) Provisional Application No. 60/784,228, filed Mar. 21, 2006;
- (2) Provisional Application No. 60/850,467, filed Oct. 10, 2006;
- (3) Provisional Application No. 60/850,681, filed Oct. 10, 2006; and
- (4) Provisional Application No. 60/881,310, filed on Jan. 19, 2007;
- (5) Provisional Application No. 60/994,344, filed Sep. 19, 2007; and
- (6) Provisional Application No. 60/994,483, filed Sep. 19, 2007.

The disclosures of the foregoing applications are incorporated herein by reference in their entireties.

**BACKGROUND**

Lyocell fibers are typically used in textiles or filter media. See, for example, U.S. Patent Application Publication No. 2003/0177909, now U.S. Pat. No. 6,872,311, and No. 2003/0168401, now U.S. Pat. No. 6,835,311, both to Koslow, as well as to U.S. Pat. No. 6,511,746 to Collier et al. On the other hand, high efficiency wipers for cleaning glass and other substrates are typically made from thermoplastic fibers.

U.S. Pat. No. 6,890,649 to Hobbs et al. (3M) discloses polyester microfibers for use in a wiper product. According to the '649 patent, the microfibers have an average effective diameter of less than 20 microns and, generally, from 0.01

microns to 10 microns. See column 2, lines 38 to 40. These microfibers are prepared by fibrillating a film surface and then harvesting the fibers.

U.S. Pat. No. 6,849,329 to Perez et al. discloses microfibers for use in cleaning wipes. These fibers are similar to those described in the '649 patent discussed above. U.S. Pat. No. 6,645,618 to Hobbs et al. also discloses microfibers in fibrous mats such as those used for removal of oil from water or those used as wipers.

5 U.S. Patent Application Publication No. 2005/0148264 to Varona et al., discloses a wiper with a bimodal pore size distribution. The wipe is made from melt blown fibers, as well as coarser fibers, and papermaking fibers. See page 2, paragraph 16.

10 U.S. Patent Application Publication No. 2004/0203306 to Grafe et al., discloses a flexible wipe including a non-woven layer and at least one adhered nanofiber layer. The nanofiber layer is illustrated in numerous photographs. It is noted on page 1, paragraph 9, that the microfibers have a fiber diameter of from about 0.05 microns to about 2 microns. In this patent application, the nanofiber webs were evaluated for cleaning automotive dashboards, automotive windows, and so forth. For example, see page 8, paragraphs 55 and 56.

15 U.S. Pat. No. 4,931,201 to Julemoni discloses a non-woven wiper incorporating melt-blown fiber. U.S. Pat. No. 4,906,513 to Kebbell et al. also discloses a wiper having melt-blown fiber. Here, polypropylene microfibers are used, and the wipers are reported to provide streak-free wiping properties. This patent is of general interest, as is U.S. Pat. No. 4,436,780 to 20 Hotchkiss et al., which discloses a wiper having a layer of melt-blown polypropylene fibers and, on either side, a spun bonded polypropylene filament layer. See also U.S. Pat. No. 4,426,417 to Meitner et al., which discloses a non-woven wiper having a matrix of non-woven fibers including microfiber and staple fiber. U.S. Pat. No. 4,307,143 to Meitner discloses a low cost wiper for industrial applications, which 25 includes thermoplastic, melt-blown fibers.

30 U.S. Pat. No. 4,100,324 to Anderson et al. discloses a non-woven fabric useful as a wiper that incorporates wood pulp fibers.

35 U.S. Patent Application Publication No. 2006/0141881, now U.S. Pat. No. 7,691,760, to Bergsten et al., discloses a wipe with melt-blown fibers. This publication also describes a drag test, at pages 7 and 9. Note, for example, page 7, paragraph 59. According to the test results on page 9, microfiber increases the drag of the wipes on a surface.

40 U.S. Patent Application Publication No. 2003/0200991 to Keck et al., discloses a dual texture absorbent web. Note pages 12 and 13, which describe cleaning tests and a Gardner wet abrasion scrub test.

45 U.S. Pat. No. 6,573,204 to Philipp et al. discloses a cleaning cloth having a non-woven structure made from micro staple fibers of at least two different polymers, and secondary staple fibers bound into the micro staple fibers. The split fiber is reported to have a titer of 0.17 to 3.0 dtex prior to being split. See column 2, lines 7 through 9. Note also, U.S. Pat. No. 6,624,100 to Pike, which discloses splittable fiber for use in microfiber webs.

**TECHNICAL FIELD**

50 This application relates to multi-ply wipers comprising at least one variable local basis weight absorbent sheet including a significant proportion of fibrillated cellulose microfiber having a plurality of arched or domed regions interconnected by a generally planar, densified fibrous network including at least some areas of consolidated fiber bordering the domed

areas. The domed regions have a leading edge with a relatively high local basis weight and, at their lower portions, transition sections that include upwardly and inwardly inflected sidewall areas of consolidated fiber.

While there have been advances in the art as to high efficiency wipers, existing products tend to be relatively difficult and expensive to produce. Many do not have the absorbent capacity of premium paper towels and are not readily repulped or recycled. Moreover, the wipers of the invention are capable of removing micro-particles and, if not substantially all of the residue from a surface, then, at least almost all, reducing the need for biocides and cleaning solutions in typical cleaning or sanitizing operations.

#### SUMMARY OF THE INVENTION

The present invention is directed, in part, to multi-ply absorbent sheets incorporating cellulose microfiber that are suitable for paper towels and wipers. The sheets exhibit high absorbency (SAT) values as well as low-residue, "wipe-dry" characteristics. The sheets can accordingly be used as high efficiency wipers, or as ordinary paper towels, eliminating the need for multiple products.

In one embodiment, the present invention is a multi-ply absorbent sheet exhibiting a wipe-dry time of less than 20 seconds, preferably, 10 seconds or less, and an SAT capacity in the range of 9.5 to 11 g/g. In a further embodiment, the absorbent sheet exhibits an SAT rate in the range of 0.05 to 0.25 g/s<sup>0.5</sup>.

A preferred variable basis weight ply is prepared by a belt-creping process including compactively dewatering a nascent web containing from about 10% to about 60% of fibrillated cellulosic microfiber, applying the dewatered web to a transfer surface with an apparently random distribution of fibers, and belt-creping the web under pressure with nip parameters selected so as to rearrange the fiber orientation and, optionally, providing local basis weight variation. The plies of this invention will exhibit a repeating structure of raised arched portions that define hollow areas on their opposite side. The raised arched portions or domes have a relatively high local basis weight interconnected with a network of densified fiber. Transition areas bridging the connecting regions and the domes include upwardly and optionally inwardly inflected consolidated fiber. Generally speaking, the furnish is selected and the steps of belt creping, applying vacuum and drying are controlled such that a dried web is formed having a plurality of fiber-enriched hollow domed regions protruding from the upper surface of the sheet, the hollow domed regions having a sidewall of a relatively high local basis weight formed along at least a leading edge thereof, and connecting regions forming a network interconnecting the fiber-enriched hollow domed regions of the sheet, wherein consolidated groupings of fibers extend upwardly from the connecting regions into the sidewalls of the fiber-enriched hollow domed regions along at least the leading edge thereof. Fibrillated cellulosic microfiber present at the surface of such consolidated groupings forms venation over the surface of the consolidated grouping, while fibrillated cellulosic microfiber present within the consolidated groupings appears to enhance the bonding and consolidation therein, both apparently contributing to an increase in very small pores in the sheet structure. Preferably, such consolidated groupings of fibers are present at least at the leading and trailing edges of the domed areas. In many cases, the consolidated groupings of fibers form saddle shaped regions extending at least partially around the domed areas, wherein a venation of cellulosic microfibers extends over the surface of the

consolidated regions. In other less consolidated regions of the ply, the fibrillated cellulosic microfibers are present as intermittently bonded fibers distributed through less consolidated regions of the ply, and intermingled with conventional paper-making fibers therein, and bonded thereto largely at crossover regions where the fibers contact.

The superior wipe-dry characteristics of the inventive products are surprising in view of the very low SAT rates observed. FIGS. 1A to 1H, 1J to 1N, and 1P to 1T are photomicrographs illustrating the microstructure at a surface of multi-ply products of the invention (FIGS. 1G, 1J, and 1L), along with a variety of somewhat similar products. It is considered to be quite surprising that such greatly improved wipe dry characteristics can be observed when apparent porosity is suppressed to the extreme shown here. Without intending to be bound by theory, it is believed that the microfiber venation seen on the surfaces of the consolidated regions in the inventive products FIGS. 1G, 1J, and 1L (formed by creping from a transfer drum using a perforated polymeric belt) provides a very slow observed SAT rate and a high capillary pressure due to a large percentage of very small, easily accessible pores, as described hereafter, as well as the large number of very small pores distributed throughout the consolidated groupings. The inventive products are remarkably efficient wipers for cleaning surfaces, leaving little, if any, residue, thus, providing streak-free cleaning that is especially desirable for glass and glossy surfaces, and much preferred for sanitation purposes. Briefly, "Wipe Dry" is the time it takes for residual Windex® original glass cleaner to evaporate from a plate after a wiper substrate is dragged across a wetted surface. Low values indicate less residual liquid that results in less streaking. Without being bound by theory, it is hypothesized that Campbell's forces draw the fibrillated cellulosic microfibers into rather intimate adhesion to the consolidated fibrous regions, so that rather than bonds being formed only at crossover points between fibers, in areas of venation, line-surface adhesion can be observed between the fibrillated cellulosic microfibers and the underlying consolidated fibrous region, creating numerous highly accessible micropores therebetween, contributing to the excellent wipe dry properties. In any event, the sheets of the present invention formed by creping from a transfer surface using perforated polymeric belts exhibit both remarkable microporosity and remarkably quick wipe dry times, while maintaining satisfactory SAT capacity. Overall, sheets that are more highly consolidated exhibit shorter wipe dry times than more open sheets.

The products of the invention also exhibit wet tensiles significantly above those of commercial towel products, but have similar SAT capacity, so that the wipe-dry characteristics endure as the product absorbs liquid. FIG. 2 shows the combined attributes of wipe-dry, absorbency, and wet strength achieved in a two-ply product of the invention. Wipe-dry times approach 10 seconds or less with a cellulosic microfiber (CMF) content of 40% as compared to 25 to 30 seconds for a conventional towel.

While exhibiting very high strength, the products of the invention also exhibit an unexpectedly high level of softness, as is appreciated from FIG. 3, which illustrates softness as a function of wet tensile and cellulosic microfiber (CMF) content. It is seen in FIG. 3 that elevated softness levels are achieved even at wet tensiles, more than twice that of conventional towel. Preferred products of the present invention will exhibit a differential pore volume for pores under 5 microns in a diameter of at least about 75 mm<sup>3</sup>/micron.

Further details and advantages will become apparent from the discussion provided hereafter.

## BRIEF DESCRIPTION OF THE DRAWINGS

The invention is described with reference to the drawings, wherein:

FIGS. 1A, 1C, and 1E illustrate cellulose microfiber (CMF) containing wipers formed by creping a nascent web from a transfer cylinder using a creping fabric and are placed for easy comparison of these to similarly formed wipers without CMF, in FIGS. 1B, 1D and 1F.

FIGS. 1G, 1J, and 1L illustrate venation on CMF containing wipers formed by creping a nascent web from a transfer cylinder using a perforated polymeric creping belt and are placed for easy comparison of those to through-air dried (TAD) formed wipers, without CMF, in FIGS. 1H, 1K, and 1M.

FIGS. 1N, 1Q, and 1S illustrate CMF containing wipers formed by conventional wet press technology and are placed for easy comparison of these to similarly formed wipers, without CMF, in FIGS. 1P, 1R and 1T.

FIG. 2 illustrates the wipe dry times of three commercially available kitchen roll towel products as compared to two ply wipers containing varying amounts of CMF formed by belt creping from a transfer cylinder using an exemplary perforated belt as described herein and illustrated in FIG. 7.

FIG. 3 illustrates the relationship among softness, wet tensile strength, and fibrillated cellulosic microfiber content in wipers.

FIG. 4 illustrates the distribution of fiber lengths in a cellulosic microfiber, which is preferred for the practice of the present invention.

FIG. 5 illustrates the extraordinarily high percentage of very long cellulosic fibers attainable with fibrillated cellulosic microfiber.

FIG. 6 illustrates the emboss pattern known as "Fantale" mentioned in Example 2.

FIG. 7 illustrates the sheet contact surface of a perforated polymeric belt mentioned in Example 1.

FIG. 8 illustrates the extrusion/intrusion porosimetry system used for measuring pore volume and pore size distribution.

FIG. 9 is a schematic diagram illustrating the interaction between the pressure plate and the sample in the apparatus for measurement of pore volume distribution.

FIG. 10 illustrates the extraordinarily high percentage of very small pores attainable in wipers comprising various amounts of fibrillated cellulosic microfibers.

FIG. 11 illustrates the relationship between wipe dry times and capillary pressure in wipers.

FIG. 12 illustrates the relationship between capillary pressure and fibrillated cellulosic microfiber content in wipers.

FIG. 13 illustrates the inter-relationship among wet tensile strength, wipe dry time, and content of fibrillated cellulosic microfiber content in a wiper.

FIG. 14 illustrates the softness of a variety of wipers as a function of GM tensile strength with fibrillated cellulosic microfiber content being indicated as a parameter.

FIG. 15 illustrates the softness of a variety of wipers as a function of cross machine direction (CD) wet tensile strength with fibrillated cellulosic microfiber content being indicated as a parameter.

FIG. 16 illustrates wipe dry times as a function of SAT capacity with fibrillated cellulosic microfiber content being indicated as a parameter.

FIG. 17 illustrates wipe dry times as a function of water holding capacity with fibrillated cellulosic microfiber content being indicated as a parameter.

FIG. 18 illustrates wipe dry times as a function of SAT rate with fibrillated cellulosic microfiber content being indicated as a parameter.

FIG. 19 illustrates wipe dry times as a function of fibrillated cellulosic microfiber content with wet strength resin content being indicated as a parameter.

FIG. 20 illustrates variation in wet extracted lint for a variety of wipers with fibrillated cellulosic microfiber content, wet strength agent content, and debonder content being indicated.

FIG. 21 illustrates the response of caliper and SAT capacity in wipers to calendering.

FIG. 22 illustrates variation in the cross machine direction (CD) wet tensile strength for a variety of towels as a function of basis weight.

FIG. 23 illustrates the response of basesheet caliper to shoe press load in a variety of wipers.

FIG. 24 illustrates basesheet caliper as a function of fibrillated cellulosic microfiber content at a constant shoe press load.

FIGS. 25A and 25B illustrate an emboss pattern known as "Little Circles" mentioned in Example 2.

FIG. 26 illustrates an emboss pattern known as "Patch-work" mentioned in Example 2.

FIG. 27 illustrates the CD wet tensile strength of a variety of towels as a function of basis weight.

FIG. 28 is a schematic scale drawing of a preferred belt usable in the practice of the present invention.

FIG. 29 illustrates the CD wet tensile strength of a variety of towels as a function of caliper.

FIG. 30 illustrates the SAT capacity of a variety of towels as a function of caliper.

FIG. 31 illustrates variation in SAT capacity for a variety of towels as a function of basis weight.

FIG. 32 illustrates the relationship between CD wet tensile strength and Sensory Softness for a variety of towels.

FIG. 33 presents SAT capacity and wipe dry times for both black glass and stainless steel surfaces for the wipers of Example 2.

FIG. 34 is a sectional scanning electron micrograph (SEM) illustrating a consolidated region in a sheet formed by belt creping using a perforated polymeric belt.

FIG. 35 is an enlarged view of a portion of FIG. 34 illustrating a domed region and a consolidated region in more detail.

FIG. 36 is a sectional scanning electron micrograph (SEM) illustrating another consolidated region in a sheet formed by belt creping using a perforated polymeric belt.

FIG. 37 compares the relative improvements in wipe dry of wipers made by creping with a woven fabric as compared to wipers made by belt creping using a perforated polymeric belt.

FIG. 38 compares wipe dry of wipers made by creping with a woven fabric as compared to wipers made by belt creping using a perforated polymeric belt.

FIG. 39 illustrates the effect of excessive quaternary ammonium salt release agent on wipers made by belt creping using a perforated polymeric belt.

FIG. 40 is an isometric schematic illustrating a device to measure roll compression of tissue products.

FIG. 41 is a sectional view taken along line 41-41 of FIG. 40.

FIG. 42 illustrates the dimensions of a marked microscope slide used in evaluating the resistance of the products of the present invention to wet linting.

#### DETAILED DESCRIPTION OF THE INVENTION

The invention is described in detail below with reference to several embodiments and numerous examples. Such a discussion is for purposes of illustration only. Modifications to particular examples within the spirit and scope of the present invention, set forth in the appended claims, will be readily apparent to one of skill in the art.

Terminology used herein is given its ordinary meaning, for example, mils refers to thousandths of an inch, mg refers to milligrams and  $m^2$  refers to square meters, percent means weight percent (dry basis), "ton" means short ton (2000 pounds), unless otherwise indicated "ream" means 3000  $ft^2$ , and so forth. A "ton" is 2000 pounds while a "tonne" is a metric ton of 100 kg or 2204.62 pounds. Unless otherwise specified, in an abbreviation "t" stands for "ton". Unless otherwise specified, the version of a test method applied is that in effect as of Jan. 1, 2010, and test specimens are prepared under standard TAPPI conditions, that is, preconditioned for 24 hours, then conditioned in an atmosphere of  $23^\circ \pm 1.0^\circ C.$  ( $73.4^\circ \pm 1.8^\circ F.$ ) at 50% relative humidity for at least about 2 hours.

Test methods, materials, equipment, manufacturing techniques, and terminology are those enumerated in the applications referred to above as supplemented herein.

Throughout this specification and claims, when we refer to a nascent web having an apparently random distribution of fiber orientation or use like terminology), we are referring to the distribution of fiber orientation that results when known forming techniques are used for depositing a furnish on the forming fabric. When examined microscopically, the fibers give the appearance of being randomly oriented, even though, depending on the jet to wire speed ratio, there may be a significant bias toward machine direction orientation making the machine direction tensile strength of the web exceed the cross machine direction tensile strength.

In many applications related to U.S. Patent Application Publication No. 2004/0238135, entitled "Fabric Crepe Process for Making Absorbent Sheet", now U.S. Pat. No. 7,399,378, the importance of the distinction between creping using a woven fabric and a creping belt formed by perforating a solid belt was of minor importance, so the term "belt" could apply to either creping medium. In this application, however, as well as in U.S. Patent Application Publication No. 2010/0186913, entitled "Belt-Creped, Variable Local Basis Weight Absorbent Sheet Prepared With Perforated Polymeric Belt", now U.S. Pat. No. 8,293,072, the distinction between the use of a creping fabric and a perforated polymeric belt is of considerable importance, as it has been found that the use of a perforated polymeric belt makes it possible to obtain consolidated regions, particularly, consolidated saddle shaped regions, in the web giving, it improved physical properties over the webs previously formed using the technique of creping from a transfer drum. For convenience, we refer to this method of forming a sheet as Fiber Reorienting Belt Creping or FRBC. Further, in this application, it is demonstrated that CMF containing wipers made using a perforated polymeric belt have substantial performance advantages over wipers made using a woven creping fabric, which we term Fiber Reorienting Fabric Creping or FRFC. Throughout this application, we have endeavored to make this distinction explicit, but, definitional language in applications incorporated by

reference notwithstanding, in this application, belts and creping fabrics should not be considered to be synonymous.

Unless otherwise specified, "basis weight", BWT, bwt, BW, and so forth, refers to the weight of a 3000 square-foot ( $278.7 m^2$ ) ream of product (basis weight is also expressed in  $g/m^2$  or gsm). Likewise, "ream" means a 3000 square-foot ( $278.7 m^2$ ) ream unless otherwise specified. Local basis weights and differences therebetween are calculated by measuring the local basis weight at two or more representative 10 low basis weight areas within the low basis weight regions and comparing the average basis weight to the average basis weight at two or more representative areas within the relatively high local basis weight regions. For example, if the representative areas within the low basis weight regions have 15 an average basis weight of 15 lbs/3000  $ft^2$  ( $24.5 g/m^2$ ) ream and the average measured local basis weight for the representative areas within the relatively high local basis regions is 20 lbs/3000  $ft^2$  ream ( $32.6 g/m^2$ ), the representative areas within the high local basis weight regions have a characteristic basis 20 weight of  $((20-15)/15) \times 100\%$  or 33% higher than the representative areas within the low basis weight regions. Preferably, the local basis weight is measured using a beta particle attenuation technique as referenced herein. In some cases, X-ray techniques can be suitable, provided that the X-rays are sufficiently "soft"—that the energy of the photons is sufficiently low and the basis weight differences between the various regions of the sheet are sufficiently high that significant differences in attenuation are attained.

Calipers and/or bulk reported herein may be measured at 8 30 or 16 sheet calipers as specified. The sheets are stacked and the caliper measurement taken about the central portion of the stack. Preferably, the test samples are conditioned in an atmosphere of  $23^\circ \pm 1.0^\circ C.$  ( $73.4^\circ \pm 1.8^\circ F.$ ) at 50% relative humidity for at least about 2 hours and then measured with a 35 Thwing-Albert Model 89-11-JR or Progage Electronic Thickness Tester with 2 in. (50.8-mm) diameter anvils, 539  $\pm$  10 grams dead weight load, and 0.231 in/sec (5.87 mm/sec) descent rate. For finished product testing, each sheet of product to be tested must have the same number of plies as 40 the product as sold. For testing in general, eight sheets are selected and stacked together. For napkin testing, napkins are unfolded prior to stacking. For base sheet testing off of winders, each sheet to be tested must have the same number of plies as produced off of the winder. For base sheet testing off of the papermachine reel, single plies must be used. Sheets are stacked together aligned in the machine direction (MD). Bulk 45 may also be expressed in units of volume/weight by dividing caliper by basis weight.

Consolidated fibrous structures are those that have been so 50 highly densified that the fibers therein have been compressed to ribbon-like structures and the void volume is reduced to levels approaching or perhaps even less than those found in flat papers, such as are used for communications purposes. In preferred structures, the fibers are so densely packed and 55 closely matted that the distance between adjacent fibers is typically less than the fiber width, often less than half or even less than a quarter of the fiber width. In the most preferred structures, the fibers are largely collinear and strongly biased in the MD. The presence of consolidated fiber or consolidated 60 fibrous structures can be confirmed by examining thin sections that have been embedded in resin, then microtomed in accordance with known techniques. Alternatively, if SEM's of both faces of a region are so heavily matted as to resemble flat paper, then that region can be considered to be consolidated. Sections prepared by focused ion beam cross section 65 polishers, such as those offered by JEOL®. 11 Dearborn Road, Peabody, Mass., 01960, are especially suitable for

observing densification throughout the thickness of the sheet, to determine whether regions in the tissue products of the present invention have been so highly densified as to become consolidated.

Creping belt, and like terminology, refers to a belt that bears a perforated pattern suitable for practicing the process of the present invention. In addition to perforations, the belt may have features, such as raised portions and/or recesses between perforations, if so desired. Preferably, the perforations are tapered, which appears to facilitate transfer of the web, especially, from the creping belt to a dryer, for example. Typically, the face of the sheet contacting the web during the fabric creping step will have a greater open area than the face away from the web. In some embodiments, the creping belt may include decorative features, such as geometric designs, floral designs, and so forth, formed by rearrangement, deletion, and/or a combination of perforations having varying sizes and shapes.

“Dome”, “domed”, “dome-like,” and so forth, as used in the description and claims, refers generally to hollow, arched protuberances in the sheet of the class seen in the various Figures, and is not limited to a specific type of dome structure as is illustrated in FIGS. 34 to 36. The terminology refers to vaulted configurations, generally, whether symmetric or asymmetric about a plane bisecting the domed area. Thus, “dome” generally refers to spherical domes, spheroidal domes, elliptical domes, ellipsoidal domes, oval domes, domes with polygonal bases, and related structures, generally including a cap and sidewalls, preferably inwardly and upwardly inclined, that is, the sidewalls being inclined toward the cap along at least a portion of their length.

#### Extractable Lint Test

To quantify the amount of lint removed from towel, tissue, and related products when used dry (“Extractable Lint”), a Sutherland Rub Tester with a 4.0-lb sled is used. This apparatus is available from: Danilee Company, 27223 Starry Mountain Street, San Antonio, Tex. 78260, 830-438-7737, 800-438-7738 (FAX). The 4.0-lb rub block for the Rub Tester has dimensions of 2" by 4", so that the pressure exerted during testing is 0.5 psi.

After the samples to be evaluated are preconditioned at 10 to 35% RH at 22° to 40° C. for 24 hours, then conditioned at 50.0%±2.0% RH and 23.0±1.0° C. for 2 hours, all of the subsequent procedures are performed within the confines of a room maintained at between 48 to 53% RH and a temperature of between 22° C. and 24° C.

Two stacks of four 2.25 in.×4.5 in. test strips with a 4.5 in. length in the machine direction are cut from the sample with the top (exterior of roll) side up.

Two 2.5 in.×6 in. strips of black felt are cut with the 6 in. length in the machine direction, and the top side labeled with sample ID numbers.

A baseline reading for the felt is determined by taking one L\* lightness color reading on the labeled side of each black felt strip used for testing in the middle of what will be the rubbed area using a GretagMacbeth® Ci5 spectrophotometer using the following settings on the spectrophotometer: Large area view, Specular component excluded, UV Source C, 2 degree observer, and Illuminant C. (In this connection, the asterisk “\*” is not a reference mark directing the reader to some other location in this document, but a portion of the commonly used symbol for CIE 1976 lightness “L\*”. “L\*” as used in this connection relates to CIE 1976, also known as CIELAB measurement of lightness, and should not be confused with Hunter lightness typically denominated “L”.) The

GretagMacbeth® spectrophotometer Model Ci5 is available from: GretagMacbeth®, 617 Little Britain Road, New Windsor, N.Y. 12553, 914-565-7660, 914-565-0390 (FAX); www.gretagmacbeth.com. The “before testing” reading is later compared to the “after testing” reading in the same area of the black felt strip on the same side, so particular care is taken to be sure that a comparison is made only between the same felt strips.

To evaluate a specimen, the specimen is taped to the galvanized plate on the Sutherland Rub Tester with the top side up, so that rubbing will be in the machine direction with care being observed to ensure that each specimen is taped in the same rub area each time the test is performed. The first black felt specimen is taped, labeled side out, to the bottom of the 4.0-lb rub block of the Sutherland Rub Tester, the number of strokes on the rub tester is set to four, and the slow speed selected (#2 setting for 4 speed model or #1 setting for 2 speed model), the rub block is placed on the Sutherland Rub Tester carriage arm and the “Start” button pressed to start testing. After the four strokes are completed, the rub block is removed from the tester and the black felt is removed from the bottom of the rub block with the black felt being preserved for L\* “after testing” color reading. The specimen is removed from the galvanized plate and discarded.

One L\* color reading is taken on the labeled side of each black felt strip, reading the same spot used to obtain the “before testing” value, in the middle of the rubbed area. The “after testing” reading is paired up with the appropriate “before testing” reading to calculate difference between the readings—“ΔL\*”.

For each sample, the average, standard deviation, minimum and maximum test results are recorded as measured to the nearest 0.01 L\* unit for both the before testing and after testing values. The difference value of the after reading minus the before reading is indicative of the lint removal by the standardized dry rubbing procedure.

#### Wet Abrasion Lint Test

Two tests are used herein to evaluate wet linting of tissue samples: in one approach, fiber is rubbed against a wetted pigskin under controlled conditions, the resulting fiber is washed off of the pigskin and the number of fibers removed is measured using an OpTest® Fiber Quality Analyzer. In the second, tissue is rubbed against wetted black felt under controlled conditions and the area of the lint left behind is measured using a flat bed scanner as described below.

#### Area Test

To evaluate a tissue sample for lint removal by wet abrasion, the sample is first subjected to simulated wet use against a sample of standard black felt with a Crockmeter Rub Tester, modified as described herein, then, the area in mm<sup>2</sup> of the lint left on the felt is measured with an Epson Perfection 4490 flat bed scanner and Apogee, SpecScan Software, version 2.3.6.

The Crockmeter Rub is available from: SDL Atlas, LLC, 3934 Airway Drive, Rock Hill, S.C. 29732, (803) 329-2110. To be used to measure wet lint as described herein, the Crockmeter is modified to accept a 360 gram arm and a 1"×2" foot that exerts a pressure on the specimen of 0.435 psi. The weight of the rub block is 355 g for the weighted arm supported on one end, and 36 g for the rub foot. These weights are exerted on a 1"×2" area, for a pressure of 391 g/12.9 cm<sup>2</sup>–30.3 g/cm<sup>2</sup>. In contrast, the method of evaluating wet abrasion in U.S. Pat. No. 5,958,187 to Bhat et al., and U.S. Pat. No.

## 11

6,059,928 to Luu et al., used a 135 g sled placed on a 2×3" sample for a pressure of 135 g/38.7 cm<sup>2</sup>=3.5 g/cm<sup>2</sup>.

Research Dimensions, at 1720 Oakridge Road, Neenah, Wis. 54956, 920-722-2289, will modify Crockmeter Rub Testers to conform hereto.

Suitable black felt is  $\frac{3}{16}$ -inch thick, part number 113308F-24 available from Aetna Felt Corporation, 2401 W. Emaus Avenue, Allentown, Pa. 18103, 800-526-4451.

To test a sample, the outer three layers of tissue are removed from the roll. Three sheets of tissue are cut at the perforations and placed in a stack using a paper cutter ensuring that the tissue sheets are placed in the same orientation relative to the direction and the side of the roll. From the stack, samples that are 2 inches by 2.5 inches are cut with the long dimension being the machine direction. Enough samples are cut for 4 replicates. The short (2') side of the tissue is marked with a small dot to indicate the surface of the tissue that was outwardly facing when on the roll. The foot is mounted to the arm of the Crockmeter with the short dimension parallel to the stroke of the Crockmeter and the stroke distance set at 4"± $\frac{1}{8}$  inch, and the stroke speed is set to ten strokes per minute. The black felt is cut into 3 inch by 6 inch pieces with the inside surface being marked along the short edge. In this test, the tissue sample to be tested will be rubbed against the inside of the felt starting at the mark. A 12 inch by 12 inch sheet of Black Acrylic, a 2 inch by 3 inch glass microscope slide marked as shown in FIG. 42, a tape, a pipette, and a beaker of distilled water are located on any nearby convenient flat surface. The Crockmeter is turned on, then turned off, to position the arm at its furthest back position. The spacer is placed under the arm to hold it above the rubbing surface. A clean piece of black felt is taped to the base of the Crockmeter over the rubbing surface with the marked surface oriented upward with the marked end up adjacent to the beginning point of the stroke of the foot. A sample is taped along one shorter edge to the foot with the top side of the tissue facing up, and the length of the tissue is wrapped around the foot and attached to the arm of the Crockmeter with the taped side and the marked location on the tissue sample facing the operator at the forward portion of the Crockmeter. The type of tape used is not critical. Office tape commonly referred to as cellophane tape or sold wider the trademark "Scotch® Tape" is suitable. The spacer is removed from under the arm and the arm with the attached foot is set down on the black felt with the long dimension of the foot perpendicular to the rub direction, and the foot is fixed in place. The glass microscope slide is placed on the felt forward of the foot and 3 volumes of 200  $\mu$ L of distilled water each are dispensed from the pipette onto the cross-marks on the glass slide. The sample, foot and arm are gently lifted, the glass slide is placed under the sample, and the sample is lowered to allow the water to wet the sample for 5 seconds, after which time the arm is lifted, the glass slide removed and the Crockmeter activated to allow the sample to make three forward strokes on the felt with the arm being lifted manually at the beginning of each return stroke to prevent the sample from contacting the felt during the return strokes. After three forward strokes, the Crockmeter is inactivated and the spacer placed under the arm so that the black felt can be removed without disturbing the abraded lint thereupon. Three minutes after the felt is removed from the rubbing surface, the felt is scanned in an Epson, Perfection 4490 flat bed scanner using Apogee SpecScan Software version 2.3.36 with the software being set for "lint" in the "Scanner Settings" window, with "2" being set in the "Process Groups of:" window on the "Defaults panel", the "Resolution" being set at "600 dots/inch", the "Scanner Mode" being set to "256-Grayscale", the "Area Setting" being set to "Special", the

## 12

"Scan Image" being set to "Reverse Image", the "Upper Limit" window on the "Dirt Histogram" panel being set to ">5.000" the "Lower Limit" window of that panel being set to "0.013-0.020" and the "X Scale:" window being set to "25"; and the "PPM" window of the "Bad Handsheet" panel set to "2500.0". On the "Printout Settings:" panel, the "Gray-Summary", "Sheet Summary" and "Gray Histogram" boxes are checked, the "Copies" window is set to "1", while the "Dirt Histogram", "Categories" and "XY Location boxes on that panel are unchecked. Both the "Enable Display" and "Enable Zoom" boxes are checked on the Display Mode panel. On the "Scanner Setup" panel, the "White" box is set for "255" while the "Black" box is set for "0", the "Contrast Filter" box is set for "0.000", the upper "Threshold=" box is set for 80.0 [% percent of background plus] while the lower "Threshold=" box is set for "0.0" [grayscale value]. The "Percent of Background, plus offset" box on the "Scanner Setup" panel is checked while the "Manual Threshold Setting" and "Function of StdDev of Background" boxes are unchecked. If desired, the "Grade Identification:" and "Reel/Load Number:" boxes may be used to record indicia related to the identification of the samples being tested. On the "Special Area Definition" panel, "Inches" is checked in the "Dimensions:" region while "Rectangular" is checked in the "Shape:" region. In the "Border at top and left:" region, "0.15" [in.] is entered in the "At the left side: (X)" box and "0.625" [in.] is entered in the "At the top: (Y)" box. In the "Area to scan:" regions "2.7" [in.] is entered in the "Width (X)" box and "5.2" [in.] is entered in the "Height (Y)" box. After scanning, the area in mm<sup>2</sup> of the abraded lint left on the black felt is output in the "SHEETS" Table in the "Total Area" column under the "Sample Sheet(s)" heading on the "Sheet & Category Summary" screen. This result is sometimes referred to herein as "WALA" for Wet Abraded Lint Area, which is reported in mm<sup>2</sup>.

## Fiber Count Test

In other cases, rather than using black felt, a pigskin comparable to human skin is substituted therefor, the fiber removed will be washed off and the solution subjected to testing in an Optest® Fiber Quality Analyzer to determine the number of fibers removed having a length in excess of 40  $\mu$ m. The Optest® Fiber Quality Analyzer has become a standard in the paper industry for determining fiber length distributions and fiber counts (above a certain minimal length, which keeps decreasing periodically, as Optest® continually upgrades their technique). The Optest® Fiber Quality Analyzer is available from:

Op Test Equipment Inc.

900 Tupper St.—Hawkesbury—ON—K6A 3S3—Canada  
Phone: 613-632-5169 Fax: 613-632-3744.

Fpm refers to feet per minute, while fps refers to feet per second.

MD means machine direction and CD means cross-machine direction.

"Predominantly" means more than 50% of the specified component, by weight unless otherwise indicated.

## 60 Roll Compression Test

Roll compression is measured by compressing roll 285 under a 1500 g flat platen 281 of a test apparatus 283 similar to that shown in FIGS. 40 and 41, then measuring the difference in height between the uncompressed roll and the compressed roll while in the fixture. Sample rolls 285 are conditioned and tested in an atmosphere of 23.0°±1.0° C.

## 13

( $73.4^{\circ}\pm1.8^{\circ}$  F.). A suitable test apparatus **283** with a movable 1500 g platen **281** (referred to as a Height Gauge) is available from:

## Research Dimensions

1720 Oakridge Road

Neenah, Wis. 54956

920-722-2289

920-725-6874 (FAX).

The test procedure is generally as follows:

(a) Raise the platen **281** and position the roll **285** to be tested on its side, centered under the platen **281**, with the tail seal **287** to the front of the gauge and the core **289** parallel to the back of the gauge **291**.

(b) Slowly lower the platen **281** until it rests on the roll **285**.

(c) Read the compressed roll diameter height from the gauge pointer **293** to the nearest 0.01 inch (0.254 mm).

(d) Raise the platen **281** and remove the roll **285**.

(e) Repeat for each roll to be tested.

To calculate roll compression in percent, the following formula is used:

$$RC(\%) = 100 \times \frac{(initial\ roll\ diameter - compressed\ roll\ diameter)}{initial\ roll\ diameter}.$$

Dry tensile strengths (MD and CD), stretch, ratios thereof, modulus, break modulus, stress and strain are measured with a standard Instron® test device or other suitable elongation tensile tester, which may be configured in various ways, typically, using 3 inch (76.2 mm) or 1 inch (25.4 mm) wide strips of tissue or towel, conditioned in an atmosphere of  $23^{\circ}\pm1^{\circ}$  C. ( $73.4^{\circ}\pm1^{\circ}$  F.) at 50% relative humidity for 2 hours. The tensile test is run at a crosshead speed of 2 in/min (50.8 mm/min). Break modulus is expressed in grams/3 inches/% strain or its SI equivalent of g/mm/% strain. % strain is dimensionless and need not be specified. Unless otherwise indicated, values are break values. GM refers to the square root of the product of the MD and CD) values for a particular product. Tensile energy absorption (TEA), which is defined as the area under the load/elongation (stress/strain) curve, is also measured during the procedure for measuring tensile strength. Tensile energy absorption is related to the perceived strength of the product in use. Products having a higher TEA may be perceived by users as being stronger than similar products that have lower TEA values, even if the actual tensile strength of the two products are the same. In fact, having a higher tensile energy absorption may allow a product to be perceived as being stronger than one with a lower TEA, even if the tensile strength of the high-TEA product is less than that of the product having the lower tensile energy absorption. When the term "normalized" is used in connection with a tensile strength, it simply refers to the appropriate tensile strength from which the effect of basis weight has been removed by dividing that tensile strength by the basis weight. In many cases, similar information is provided by the term "breaking length".

Tensile ratios are simply ratios of the values determined by way of the foregoing methods. Unless otherwise specified, a tensile property is a dry sheet property.

"Upper", "upwardly" and like terminology is used purely for convenience and does not require that the sheet be placed in a specified orientation, but rather, refers to position or direction toward the caps of the dome structures, that is, the belt side of the web, which is generally opposite to the Yankee side, unless the context clearly indicates otherwise.

## 14

"Venation" means a structure presenting a generally smooth surface having raised, generally continuous ridges defined thereacross, similar to the venation observable on the lower surface of many common leaves.

5 The void volume and/or void volume ratio, as referred to hereafter, are determined by saturating a sheet with a nonpolar POROFIL™ liquid, available from Coulter Electronics Ltd. (Beckman Coulter, Inc. 250 S. Kraemer Boulevard, P.O. Box 8000, Brea, Calif. 92822-8000 USA, Part No. 9902458), and measuring the amount of liquid absorbed. The volume of liquid absorbed is equivalent to the void volume within the sheet structure. The % weight increase (PWI) is expressed as grams of liquid absorbed per grain of fiber in the sheet structure times one hundred, as noted hereafter. More specifically, 10 for each single-ply sheet sample to be tested, select 8 sheets and cut out a 1 inch by 1 inch (25.4 mm by 25.4 mm) square (1 inch (25.4 mm) in the machine direction and 1 inch (25.4 mm) in the cross machine direction). For multi-ply product samples, each ply is measured as a separate entity. Multiple samples should be separated into individual single plies and 15 8 sheets from each ply position used for testing. Weigh and record the dry weight of each test specimen to the nearest 0.0001 gram. Place the specimen in a dish containing POROFIL™ liquid having a specific gravity of about 1.93 grams per cubic centimeter. After 10 seconds, grasp the specimen at the very edge (1 to 2 millimeters in) of one corner with tweezers and remove from the liquid. Hold the specimen with that corner uppermost and allow excess liquid to drip for 30 seconds. Lightly dab (less than  $\frac{1}{2}$  second contact) the lower 20 corner of the specimen on #4 filter paper (Whatman Ltd., Maidstone, England) in order to remove any excess of the last partial drop. Immediately weigh the specimen, within 10 seconds, recording the weight to the nearest 0.0001 gram. The PWI for each specimen, expressed as grams of POROFIL™ liquid per gram of fiber, is calculated as follows:

$$PWI = [(W_2 - W_1) / W_1] \times 100,$$

wherein

" $W_1$ " is the dry weight of the specimen, in grains; and

" $W_2$ " is the wet weight of the specimen, in grams.

30 The PWI for all eight individual specimens is determined as described above and the average of the eight specimens is the PWI for the sample.

The void volume ratio is calculated by dividing the PWI by 45 1.9 (density of fluid) to express the ratio as a percentage, whereas the void volume (gms/gm) is simply the weight increase ratio, that is, PWI divided by 100.

50 Water absorbency rate is related to the time it takes for a sample to absorb a 0.1 gram droplet of water disposed on its surface by way of an automated syringe. The test specimens are preferably conditioned at  $23^{\circ}$  C.  $\pm 1^{\circ}$  C. ( $73.4^{\circ}$  F.  $\pm 1^{\circ}$  F.) at 50% relative humidity. For each sample, four 3x3 inch test specimens are prepared. Each specimen is placed in a sample holder such that a high intensity lamp is directed toward the 55 specimen. 0.1 ml of water is deposited on the specimen surface and a stop watch is started. When the water is absorbed, as indicated by lack of further reflection for light from the drop, the stopwatch is stopped and the time is recorded to the nearest 0.1 seconds. The procedure is repeated for each specimen and the results averaged for the sample. SAT rate is determined by graphing the weight of water absorbed by the sample (in grams) against the square root of time (in seconds). The SAT rate is the best fit slope between 10 and 60 percent of the end point (grams of water absorbed), and is expressed in 60 g/s<sup>0.5</sup>.

65 The wet tensile of a wiper of the present invention is measured generally following TAPPI Method T 576 pm-07 using

## 15

a three-inch (76.2 mm) wide strip of tissue that is folded into a loop, clamped in a special fixture termed a Finch Cup, then immersed in water. A suitable Finch cup, 3 inch (76.2 mm), with base to fit a 3 inch (76.2 mm) grip, is available from:

High-Tech Manufacturing Services, Inc.  
3105-B NE 65<sup>th</sup> Street  
Vancouver, Wash. 98663  
360-696-1611  
360-696-9887 (FAX).

For fresh basesheet and finished product (aged 30 days or less for towel product, aged 24 hours or less for tissue product) containing wet strength additive, the test specimens are placed in a forced air oven heated to 105° C. (221° F.) for five minutes. No oven aging is needed for other samples. The Finch cup is mounted onto a tensile tester equipped with a 2.0 pound (8.9 Newton) load cell with the flange of the Finch cup clamped by the tester's lower jaw and the ends of tissue loop clamped into the upper jaw of the tensile tester. The sample is immersed in water that has been adjusted to a pH of 7.01±0.1 and the tensile is tested after a 5 second immersion time using a crosshead speed of 2 inches/minute (50.8 mm/minute). The results are expressed in g/3 in. or (g/mm), dividing the readout by two to account for the loop as appropriate.

Wipe dry times are evaluated using a turntable wipe dry instrument with a spray fluid dispensing instrument, each being as described below. For purposes of this application, two standard test surfaces are used: stainless steel and black glass. To evaluate a sample, the paper is first pre-conditioned and conditioned as described below, the test surface cleaned with Windex® original glass cleaner from S.C. Johnson and Son, Racine, Wis., and then wiped dry with a lint-free wipe.

The test sample is folded so that the fold extends in the cross machine direction and centered on the black foam side of the sample head, so that the machine direction runs perpendicular to the shaft (i.e., the machine direction is parallel to the directions of motion) and taped in position at its corners so that the sample's leading edge is the folded edge and the towel sample is flush with the right hand edge of the sample head. The sample head is placed on the test surface and the slack in the sample removed. Windex® original glass cleaner is sprayed on the test surface in an amount of 0.75±0.1 grains in the center of the area not occupied by the test head. The table is rotated for 3 revolutions at 30 to 32 rpm with the head in engagement with the test surface at a load of 1065 g spread over bearing surface dimensions of 23 cm×9.5 cm. After the turntable has made three revolutions, the area on the test surface to which the Windex® original glass cleaner was applied is observed and the elapsed time recorded until all of the Windex® original glass cleaner has evaporated. This time is recorded in seconds as the Wipe Dry Time.

To quantify the amount of lint removed from towel, tissue, and related products (Extractable Lint), a Sutherland Rub Tester with 4.0-lb rub block is used. This is discussed above.

After the samples to be evaluated are preconditioned at 10 to 35% RH at 22° to 40° C. for 24 hours, then conditioned at 50.0%±2.0% RH and 23.0±1.0° C. for 2 hours, all of the subsequent procedures are performed within the confines of a room maintained at between 48 to 53% RH and a temperature of between 22° C. and 24° C.

Two stacks of four 2.25 in.×4.5 in. test strips with 4.5 in. length in the machine direction are cut from the sample with the top (exterior of roll) side up.

Two 2.5 in.×6 in. strips of black felt are cut with the 6 in. length in the machine direction, and the top side labeled with sample ID numbers.

A baseline reading for the felt is determined by taking one L\* color reading on the labeled side of each black felt strip

## 16

used for testing in the middle of what will be the rubbed area using a GretagMacbeth Spectrophotometer Model Ci5 as discussed above. The "before testing" reading is later compared to the "after testing" reading in the same area of the black felt strip on the same side, so particular care is taken to be sure that comparison are made only between the same felt strips.

One L\* color reading is taken on the labeled side of each black felt strip, reading the same spot used to obtain the "before testing" value, in the middle of the rubbed area. The "after testing" reading is paired up with the appropriate "before testing" reading to calculate the difference between the two readings—"ΔL\*".

For each sample, the average, standard deviation, minimum and maximum test results are recorded as measured to the nearest 0.01 L\* unit for both the before testing and after testing values. The difference value of the after reading minus the before reading is indicative of the lint removal by the standardized rubbing procedure.

## Liquid Porosimetry

Liquid porosimetry is a procedure for determining the pore volume distribution (PVD) within a porous solid matrix. Each pore is sized according to its effective radius, and the contribution of each size to the total free volume is the principal objective of the analysis. The data reveals useful information about the structure of a porous network, including absorption and retention characteristics of a material.

The procedure generally requires quantitative monitoring of the movement of liquid either into or out of a porous structure. The effective radius R of a pore is operationally defined by the Laplace equation:

$$R = \frac{2\gamma\cos\theta}{\Delta P}$$

where  $\gamma$  is liquid surface tension,  $\theta$  is advancing or receding contact angle of the liquid, and  $\Delta P$  is pressure difference across the liquid/air meniscus. For liquid to enter or to drain from a pore, an external pressure must be applied that is just enough to overcome the Laplace  $\Delta P$ .  $\cos\theta$  is negative when liquid must be forced in,  $\cos\theta$  is positive when it must be forced out. If the external pressure on a matrix having a range of pore sizes is changed, either continuously or in steps, filling or emptying will start with the largest pore and proceed in turn down to the smallest size that corresponds to the maximum applied pressure difference. Porosimetry involves recording the increment of liquid that enters or leaves with each pressure change and can be carried out in the extrusion mode, that is, liquid is forced out of the porous network rather than into it. The receding contact angle is the appropriate term in the Laplace relationship, and any stable liquid that has a known  $\cos\theta > 0$  can be used. If necessary, initial saturation with liquid can be accomplished by preevacuation of the dry material. The basic arrangement used for extrusion porosimetry measurements is illustrated in FIG. 8. The presaturated specimen is placed on a microporous membrane which is itself supported by a rigid porous plate. The gas pressure within the chamber is increased in steps, causing liquid to flow out of some of the pores, the largest ones first. The amount of liquid removed is monitored by the top-loading recording balance. In this way, each level of applied pressure (which determines the largest effective pore size that remains filled) is related to an increment of liquid mass. The chamber is pressurized by

means of a computer-controlled, reversible, motor-driven piston/cylinder arrangement that can produce the required changes in pressure to cover a pore radius range from 1 to 1000  $\mu\text{m}$ .

Eight finished product samples were analyzed for pore volume distribution testing. Measurements were performed on the TRI/Autoporusimeter®. The instrument and the PVD methodology are described in the paper “Liquid Porosimetry: New Methodology and Applications” by Dr. B. Miller and Dr. I. Tyomkin, published in the Journal of Colloid and Interface Science, 162, 163-170, (1994), the disclosure of which is incorporated herein by reference.

The test liquid was 0.1% TX-100 solution in water, surface tension 30 mN/m. TX-100 is a surfactant. For reference, water at room temperature has a sum lace tension of 72 dyne/cm. Sample size was 30  $\text{cm}^2$ . The test started in an advancing mode and finished in a receding mode. The advancing mode requires good contact with fine porous membrane in the test chamber. Therefore, samples were covered with a multi-pin plate as shown in FIG. 9. The pin plate area is 30  $\text{cm}^2$ . It has 196 0.9 $\times$ 0.9 mm square pins, the height of each pin is 4 mm, the distance between pins is 3.2 mm, and the total area of pins is 159  $\text{mm}^2$ . The pin plate locally compressed the sample. The total area of the pins is 5% of sample.

Data from 1 micron to 500 microns represent the advancing part of the curve, and data from 500 microns to 1 micron represent the receding part of the curve. At the end of the test at 1 micron, there was some liquid left in the sample. This liquid is a sum of liquid in swollen fibers, liquid in pores below 1 micron, and liquid trapped in the larger pores. The amount of liquid in a sample at the end of experiment was usually below 0.5  $\text{mm}^3/\text{mg}$ .

Water Holding Capacity is determined pursuant to withdrawn ASTM Standard Method D-4250-92, Standard Method for Water-Holding Capacity of Bibulous Fibrous Products. It is considered to be generally very comparable to SAT.

#### Regenerated Cellulose Microfiber

In accordance with the invention, regenerated cellulose fiber is prepared from a cellulosic dope comprising cellulose dissolved in a solvent comprising tertiary amine N-oxides or ionic liquids. The solvent composition for dissolving cellulose and preparing underderivatized cellulose dopes suitably includes tertiary amine oxides, such as N-methylmorpholine-N-oxide (NMMO), and similar compounds enumerated in U.S. Pat. No. 4,246,221 to McCorsley, the disclosure of which is incorporated herein by reference. Cellulose dopes may contain non-solvents for cellulose such as water, alkanols or other solvents, as will be appreciated from the discussion that follows.

Suitable cellulosic dopes are enumerated in Table 1, below.

TABLE 1

| EXAMPLES OF TERTIARY AMINE N-OXIDE SOLVENTS                 |            |             |
|-------------------------------------------------------------|------------|-------------|
| Tertiary Amine N-oxide                                      | % water    | % cellulose |
| N-methylmorpholine N-oxide                                  | up to 22   | up to 38    |
| N,N-dimethyl-ethanol-amine N-oxide                          | up to 12.5 | up to 31    |
| N,N-dimethylcyclohexylamine N-oxide                         | up to 21   | up to 44    |
| N-methylhomopiperidine N-oxide                              | 5.5-20     | 1-22        |
| N,N,N-triethylamine N-oxide                                 | 7-29       | 5-15        |
| 2(2-hydroxypropoxy)-N-ethyl-N,N,-dimethyl-<br>amide N-oxide | 5-10       | 2-7.5       |

TABLE 1-continued

| EXAMPLES OF TERTIARY AMINE N-OXIDE SOLVENTS |            |             |
|---------------------------------------------|------------|-------------|
| Tertiary Amine N-oxide                      | % water    | % cellulose |
| N-methylpiperidine N-oxide                  | up to 17.5 | 5-17.5      |
| N,N-dimethylbenzylamine N-oxide             | 5.5-17     | 1-20        |

See, also, U.S. Pat. No. 3,508,941 to Johnson, the disclosure of which is incorporated herein by reference.

Details with respect to preparation of cellulosic dopes including cellulose dissolved in suitable ionic liquids and cellulose regeneration therefrom are found in U.S. Patent Application Publication No. 2003/0157351, now U.S. Pat. No. 6,824,599, of Swatloski et al., entitled “Dissolution and Processing of Cellulose Using Ionic liquids”, the disclosure of which is incorporated herein by reference. Here again, suitable levels of non-solvents for cellulose may be included. This patent generally describes a process of dissolving cellulose in an ionic liquid without derivatization and regenerating the cellulose in a range of structural forms. It is reported that the cellulose solubility and the solution properties can be controlled by the selection of ionic liquid constituents with small cations and halide or pseudohalide anions favoring solution. Preferred ionic liquids for dissolving cellulose include those with cyclic cations, such as the following cations: imidazolium; pyridinium; pyridazinium; pyrimidinium; pyrazinium; pyrazolium; oxazolium; 1,2,3-triazolium; 1,2,4-triazolium; thiazolium; piperidinium; pyrrolidinium; quinolinium; and isoquinolinium.

Processing techniques for ionic liquids/cellulose dopes are also discussed in U.S. Pat. No. 6,808,557 to Holbrey et al., entitled “Cellulose Matrix Encapsulation and Method”, the disclosure of which is incorporated herein by reference. Note also, U.S. Patent Application Publication No. 2005/0288484, now U.S. Pat. No. 7,888,412, of Holbrey et al., entitled “Polymer Dissolution and Blend Formation in Ionic Liquids”, as well as U.S. Patent Application Publication No. 2004/0038031, now U.S. Pat. No. 6,808,557, of Holbrey et al., entitled “Cellulose Matrix Encapsulation and Method”, the disclosures of which are incorporated herein by reference. With respect to ionic fluids, in general, the following documents provide further detail: U.S. Patent Application Publication No. 2006/0241287, now U.S. Pat. No. 7,763,715, of Hecht et al., entitled “Extracting Biopolymers From a Biomass Using Ionic Liquids”; U.S. Patent Application Publication No. 2006/0240727 of Price et al., entitled “Ionic Liquid Based Products and Method of Using The Same”; U.S. Patent Application Publication No. 2006/0240728 of Price et al., entitled “Ionic Liquid Based Products and Method of Using the Same”; U.S. Patent Application Publication No. 2006/0090271 of Price et al., entitled “Processes For Modifying Textiles Using Ionic Liquids”; and U.S. Patent Application Publication No. 2006/0207722 of Amano et al., entitled “Pressure Sensitive Adhesive Compositions, Pressure Sensitive Adhesive Sheets and Surface Protecting Films,” now U.S. Pat. No. 8,318,859, the disclosures of which are incorporated herein by reference. Some ionic liquids and quasi-ionic liquids that may be suitable are disclosed by Imperato et al., Chemical Communications 2005, pages 1170 to 1172, the disclosure of which is incorporated herein by reference.

“Ionic liquid”, refers to a molten composition including an ionic compound that is preferably a stable liquid at temperatures of less than 100° C. at ambient pressure. Typically, such liquids have a very low vapor pressure at 100° C., less than 75 mBar or so, and preferably, less than 50 mBar or less than 25 mBar at 100° C. Most suitable liquids will have a vapor pressure of less than 10 mBar at 100° C., and often, the vapor pressure is so low that it is negligible, and is not easily measurable, since it is less than 1 mBar at 100° C.

19

Suitable commercially available ionic liquids are Basiionic™ ionic liquid products available from BASF (Florham Park, N.J.) and are listed in Table 2 below.

20

Fibrillated lyocell or its equivalent has advantages over splittable meltspun fibers. Synthetic microdenier fibers come in a variety of forms. For example, a 3 denier nylon/PET fiber

TABLE 2

| Exemplary Ionic Liquids         |                  |                                                    |              |
|---------------------------------|------------------|----------------------------------------------------|--------------|
| IL Abbreviation                 | Basiionic™ Grade | Product name                                       | CAS Number   |
| STANDARD                        |                  |                                                    |              |
| EMIM Cl                         | ST 80            | 1-Ethyl-3-methylimidazolium chloride               | 65039-09-0   |
| EMIM                            | ST 35            | 1-Ethyl-3-methylimidazolium methanesulfonate       | 145022-45-3  |
| CH <sub>3</sub> SO <sub>3</sub> |                  |                                                    |              |
| BMIM Cl                         | ST 70            | 1-Butyl-3-methylimidazolium chloride               | 79917-90-1   |
| BMIM                            | ST 78            | 1-Butyl-3-methylimidazolium methanesulfonate       | 342789-81-5  |
| CH <sub>3</sub> SO <sub>3</sub> |                  |                                                    |              |
| MTBS                            | ST 62            | Methyl-tri-n-butylammonium methylsulfate           | 13106-24-6   |
| MMMPZ                           | ST 33            | 1,2,4-Trimethylpyrazolium methylsulfate            |              |
| MeOSO <sub>3</sub>              |                  |                                                    |              |
| EMMIM                           | ST 67            | 1-Ethyl-2,3-di-methylimidazolium ethylsulfate      | 516474-08-01 |
| EtOSO <sub>3</sub>              |                  |                                                    |              |
| MMMIM                           | ST 99            | 1,2,3-Trimethyl-imidazolium methylsulfate          | 65086-12-6   |
| MeOSO <sub>3</sub>              |                  |                                                    |              |
| ACIDIC                          |                  |                                                    |              |
| HMIM Cl                         | AC 75            | Methylimidazolium chloride                         | 35487-17-3   |
| HMIM HSO <sub>4</sub>           | AC 39            | Methylimidazolium hydrogensulfate                  | 681281-87-8  |
| EMIM HSO <sub>4</sub>           | AC 25            | 1-Ethyl-3-methylimidazolium hydrogensulfate        | 412009-61-1  |
| EMIM AlCl <sub>4</sub>          | AC 09            | 1-Ethyl-3-methylimidazolium tetrachloroaluminate   | 80432-05-9   |
| BMIM HSO <sub>4</sub>           | AC 28            | 1-Butyl-3-methylimidazolium hydrogensulfate        | 262297-13-2  |
| BMIM AlCl <sub>4</sub>          | AC 01            | 1-Butyl-3-methylimidazolium tetrachloroaluminate   | 80432-09-3   |
| BASIC                           |                  |                                                    |              |
| EMIM Acetat                     | BC 01            | 1-Ethyl-3-methylimidazolium acetate                | 143314-17-4  |
| BMIM Acetat                     | BC 02            | 1-Butyl-3-methylimidazolium acetate                | 284049-75-8  |
| LIQUID AT RT                    |                  |                                                    |              |
| EMIM EtOSO <sub>3</sub>         | LQ 01            | 1-Ethyl-3-methylimidazolium ethylsulfate           | 342573-75-5  |
| BMIM MeOSO <sub>3</sub>         | LQ 02            | 1-Butyl-3-methylimidazolium methylsulfate          | 401788-98-5  |
| LOW VISCOSITY                   |                  |                                                    |              |
| EMIM SCN                        | VS 01            | 1-Ethyl-3-methylimidazolium thiocyanate            | 331717-63-6  |
| BMIM SCN                        | VS 02            | 1-Butyl-3-methylimidazolium thiocyanate            | 344790-87-0  |
| FUNCTIONALIZED                  |                  |                                                    |              |
| COL Acetate                     | FS 85            | Choline acetate                                    | 14586-35-7   |
| COL Salicylate                  | FS 65            | Choline salicylate                                 | 2016-36-6    |
| MTEOA                           | FS 01            | Tris-(2-hydroxyethyl)-methylammonium methylsulfate | 29463-06-7   |
| MeOSO <sub>3</sub>              |                  |                                                    |              |

Cellulose dopes, including ionic liquids having dissolved therein about 5% by weight underivatized cellulose, are commercially available from Aldrich. These compositions utilize alkyl-methylimidazolium acetate as the solvent. It has been found that choline-based ionic liquids are not particularly suitable for dissolving cellulose.

After the cellulosic dope is prepared, it is spun into fiber, fibrillated and incorporated into absorbent sheet, as described later.

A synthetic cellulose, such as lyocell, is split into micro- and nano-fibers, and added to conventional wood pulp. The fiber may be fibrillated in an unloaded disk refiner, for example, or any other suitable technique including using a PFI beater mill. Preferably, relatively short fiber is used, and the consistency kept low during fibrillation. The beneficial features of fibrillated lyocell include biodegradability, hydrogen bonding, dispersibility, repulpability, and smaller microfibers than obtainable with meltspun fibers, for example.

50 in a so-called pie wedge configuration can be split into 16 or 32 segments, typically, in a hydroentangling process. Each segment of a 16-segment fiber would have a coarseness of about 2 mg/100 m versus eucalyptus pulp at about 7 mg/100 m. 55 Unfortunately, a number of deficiencies has been identified with this approach for conventional wet laid applications. Dispersibility is less than optimal. Melt spun fibers must be split before sheet formation, and an efficient method is lacking. Most available polymers for these fibers are not biodegradable. The coarseness is lower than that of wood pulp, but still high enough that they must be used in substantial amounts and form a costly part of the furnish. Finally, the lack of hydrogen bonding requires other methods of retaining the fibers in the sheet.

56 Fibrillated lyocell has fibrils that can be as small as 0.1 to 0.25 microns (μm) in diameter, translating to a coarseness of 0.0013 to 0.0079 mg/100 m. Assuming these fibrils are available as individual strands—separate from the parent fiber—

the furnish fiber population can be dramatically increased at various addition rates. Even fibrils not separated from the parent fiber may provide benefit. Dispersibility, repulpability, hydrogen bonding, and biodegradability remain product attributes since the fibrils are cellulose.

Fibrils from lyocell fiber have important distinctions from wood pulp fibrils. The most important distinction is the length of the lyocell fibrils. Wood pulp fibrils are only perhaps microns long, and, therefore, act in the immediate area of a fiber-fiber bond. Wood pulp fibrillation from refining leads to stronger, denser sheets. Lyocell fibrils, however, are potentially as long as the parent fibers. These fibrils can act as independent fibers and improve the bulk, while maintaining or improving strength. Southern pine and mixed southern hardwood (MSHW) are two examples of fibers that are disadvantaged relative to premium pulps with respect to softness. The term "premium pulps" used herein refers to northern softwoods and eucalyptus kraft pulps commonly used in the tissue industry for producing the softest bath, facial, and towel grades. Southern pine is coarser than northern softwood kraft, and mixed southern hardwood is both coarser and higher in fines than market eucalyptus. The lower coarseness and lower fines content of premium market pulp leads to a higher fiber population, expressed as fibers per gram (N or  $N_{>0.2}$ ) in Table 3. The coarseness and length values in Table 3 were obtained with an OpTest Fiber Quality Analyzer. Definitions are as follows:

$$L_n = \frac{\sum_{\text{all fibers}} n_i L_i}{\sum_{\text{all fibers}} n_i}$$

$$L_{n,i>0.2} = \frac{\sum_{i>0.2} n_i L_i}{\sum_{i>0.2} n_i}$$

$$C = 10^5 \times \frac{\text{sample weight}}{\sum_{\text{all fibers}} n_i L_i}$$

$$N = \frac{100}{CL} [= \text{million fibers/gram}]$$

Northern bleached softwood kraft (NBSK) and eucalyptus have more fibers per gram than do southern pine and hardwood. Lower coarseness leads to higher fiber populations and smoother sheets.

TABLE 3

| Fiber Properties                    |            |             |          |            |         |                  |                         |
|-------------------------------------|------------|-------------|----------|------------|---------|------------------|-------------------------|
| Sample                              | Type       | C, mg/100 m | Fines, % | $L_{n,mm}$ | N, MM/g | $L_{n,i>0.2,mm}$ | $N_{>0.2}, \text{MM/g}$ |
| Southern HW                         | Pulp       | 10.1        | 21       | 0.28       | 35      | 0.91             | 11                      |
| Southern HW - low fines             | Pulp       | 10.1        | 7        | 0.54       | 18      | 0.94             | 11                      |
| Aracruz <i>Eucalyptus</i>           | Pulp       | 6.9         | 5        | 0.50       | 29      | 0.72             | 20                      |
| Southern SW                         | Pulp       | 18.7        | 9        | 0.60       | 9       | 1.57             | 3                       |
| Northern SW                         | Pulp       | 14.2        | 3        | 1.24       | 6       | 1.74             | 4                       |
| Southern (30 SW/70 HV)              | Base sheet | 11.0        | 18       | 0.31       | 29      | 0.93             | 10                      |
| 30 Southern SW/70 <i>Eucalyptus</i> | Base sheet | 8.3         | 7        | 0.47       | 26      | 0.77             | 16                      |

For comparison, the "parent" or "stock" fibers of unfibrillated lyocell have a coarseness 16.6 mg/100 m before fibrillation and a diameter of about 11 to 12  $\mu\text{m}$ .

The fibrils of fibrillated lyocell have a coarseness on the order of 0.001 to 0.008 mg/100 m. Thus, the fiber population can be dramatically increased at relatively low addition rates. FIG. 4 illustrates the distribution of fiber lengths found in a regenerated cellulosic microfiber, which is preferred for the practice of the present invention. Fiber length of the parent fiber is selectable, and fiber length of the fibrils can depend on the starting length and the degree of cutting during the fibrillation process, as can be seen in FIG. 5.

The dimensions of the fibers passing the 200 mesh screen are on the order of 0.2 micron by 100 micron long. Using these dimensions, one calculates a fiber population of 200 billion fibers per gram. For perspective, southern pine might be three million fibers per gram and eucalyptus might be twenty million fibers per gram (Table 3). It appears that these fibers are the fibrils that are broken away from the original unrefined fibers. Different fiber shapes with lyocell intended to readily fibrillate could result in 0.2 micron diameter fibers that are perhaps 1000 microns or more long, instead of 100. As noted above, fibrillated fibers of regenerated cellulose may be made by producing "stock" fibers having a diameter of 10 to 12 microns, or so, followed by fibrillating the parent fibers. Alternatively, fibrillated lyocell microfibers have recently become available from Engineered Fibers Technology (Shelton, Conn.) having suitable properties.

Particularly preferred materials contain more than 40% fiber that is finer than 14 mesh and exhibit a very low coarseness (low freeness). For ready reference, mesh sizes appear in Table 4, below.

TABLE 4

| 35 | Mesh Size    |        |         |
|----|--------------|--------|---------|
|    | Sieve Mesh # | Inches | Microns |
| 40 | 14           | .0555  | 1400    |
|    | 28           | .028   | 700     |
|    | 60           | .0098  | 250     |
|    | 100          | .0059  | 150     |
|    | 200          | .0029  | 74      |

45 Details as to fractionation using the Bauer-McNutt Classifier appear in Gooding et al., "Fractionation in a Bauer-McNutt

Classifier", *Journal of Pulp and Paper Science*. Vol. 27. No. 12, December 2001, the disclosure of which is incorporated herein by reference. A particularly preferred microfiber is shown in Table 4A.

TABLE 4A

| Fiber Length Distribution of Preferred Regenerated Cellulosic Microfiber |          |
|--------------------------------------------------------------------------|----------|
| Fiber Length                                                             | Weight % |
| +14 mesh                                                                 | 2.3%     |
| 28 mesh                                                                  | 20.5%    |
| 48 mesh                                                                  | 10.6%    |
| 100 mesh                                                                 | 15.6%    |
| 200 mesh                                                                 | 17.2%    |
| <200 mesh                                                                | 33.8%    |

FIG. 5 is a plot showing fiber length as measured by a Fiber Quality Analyzer (FQA) for various samples of regenerated cellulosic microfiber. From this data, it is appreciated that much of the fine fiber is excluded by the FQA and length prior to fibrillation has an effect on fineness. The Optest Fiber Quality Analyzer has become a standard in the paper industry for determining fiber length distributions and fiber counts (above a certain minimum length that keeps decreasing steadily as Optest continually upgrades their technology). The OpTest Fiber Quality Analyzer is available from:

OpTest Equipment Inc.

900 Tupper St.—Hawkesbury—ON—K6A 3S3—Canada  
Phone: 613-632-5169 Fax: 613-632-3744.

#### EXAMPLE 1

##### Perforated Polymeric Belt Creping

A series of belt-creped base-sheets was prepared with the materials and layering described in Table 5, with the CMF having the approximate fiber length distribution shown in FIG. 4.

TABLE 5

| Cell | NBSK % | CMF % | Base-sheet Cells |             |               | Layered | Comments                                  |
|------|--------|-------|------------------|-------------|---------------|---------|-------------------------------------------|
|      |        |       | BW<br>lb/R       | CMC<br>lb/t | Amres<br>lb/t |         |                                           |
| 1    | 100    | 0     | 14               | 0           | 12            | No      | Control, balanced charge                  |
| 2    | 80     | 20    | 14               | 0           | 12            | No      | 20% CMF, two-ply towel                    |
| 3    | 60     | 40    | 14               | 0           | 12            | No      | 40% CMF, two-ply towel                    |
| 4    | 40     | 60    | 14               | 0           | 12            | No      | 60% CMF, two-ply towel                    |
| 5    | 100    | 0     | 14               | 12          | 40            | No      | Control, high resin                       |
| 6    | 80     | 20    | 14               | 12          | 40            | No      | 20% CMF, two-ply towel, high wet          |
| 7    | 60     | 40    | 14               | 12          | 40            | No      | 40% CMF, two-ply towel, high wet          |
| 8    | 40     | 60    | 14               | 12          | 40            | No      | 60% CMF, two-ply towel, high wet          |
| 9    | 60     | 40    | 14               | 12          | 40            | Yes     | 100% CMF on surface                       |
| 10   | 60     | 40    | 14               | 12          | 40            | Yes     | 100% CMF on surface, calender             |
| 11   | 40     | 60    | 14               | 12          | 40            | No      | High wet/dry 3 lb/t GP-C in MC 1 and MC 2 |
| 12   | 40     | 60    | 14               | 12          | 40            | No      | High wet/dry 3 lb/t GP-C, calender        |
| 13   | 60     | 40    | 14               | 12          | 40            | No      | High wet/dry 3 lb/t GP-C in MC 1 and MC 2 |

100% NBSK was delivered from a first machine chest. 100% CMF was supplied from a second machine chest. The softwood fiber was refined an average of 2.2 HPD/ton based on total flow, requiring less refined horsepower as softwood

fiber content decreased. The average freeness of the softwood fiber across the trial was 541 ml CSF.

Amres® HP 100, from Georgia-Pacific Resins, Inc., was split proportionally to the suction of each machine chest pump. Amtex Gelycel® carboxymethylcellulose (CMC) was split proportionally to the static mixer or stuff box. Titratable charge averaged 0.02 ml/10 ml for cells with no CMC and 12 lb/ton Amres®. Titratable charge averaged -0.17 ml/10 ml for cells with 12 lb/ton CMC and 40 lb/ton Amres®.

10 Trial speed averages appear in Table 6:

TABLE 6

| Trial Speed Averages |                        |      |
|----------------------|------------------------|------|
| 15                   | Jet Speed, fpm         | 2450 |
|                      | Form Roll Speed, fpm   | 1574 |
|                      | Small Dryer Speed, fpm | 1559 |
|                      | Yankee Speed, fpm      | 1251 |
|                      | Reel Speed, fpm        | 1190 |
| 20                   | Jet/Wire Ratio         | 1.56 |
|                      | Fabric Crepe Ratio     | 1.25 |
|                      | Reel Crepe Ratio       | 1.05 |
|                      | Total Crepe Ratio      | 1.31 |

25 A perforated polymer creping belt was used as described in U.S. Patent Application Publication No. 2010/0186013, entitled "Belt-Creped, Variable Local Basis Weight Absorbent Sheet Prepared With Perforated Polymeric Belt", the disclosure of which is incorporated herein by reference. The sheet contact surface of the perforated polymeric belt is illustrated in FIG. 7.

30 The basesheets produced had the properties set forth in Table 7. Base-sheets were converted to two-ply sheet using Fantale emboss pattern, FIG. 6, with a THVS configuration, that is, the pattern is embossed into only one of the two plies, which is joined to the non-embossed ply by glue lamination in 35 points to the inside configuration, such that the outer surface of the embossed ply is debossed, and the asperities created by embossing bear against and are shielded by the unembossed ply.

TABLE 7

| Roll  | CMF Percent | Amres ®, lb/t | Caliper 8 Sheet mils/8 sht | Basis Weight lb/3000 ft <sup>2</sup> | MD Tensile g/3 in. | MD Stretch % | CD Tensile g/3 in. | CD Stretch % | CD Wet     |               | SAT Capacity g/m <sup>2</sup> | GM Tensile g/3 in. | GM Break Modulus gms/% | CD Tensile Wet/Dry Unitless |
|-------|-------------|---------------|----------------------------|--------------------------------------|--------------------|--------------|--------------------|--------------|------------|---------------|-------------------------------|--------------------|------------------------|-----------------------------|
|       |             |               |                            |                                      |                    |              |                    |              | Tens Finch | Cured g/3 in. |                               |                    |                        |                             |
| 22989 | 0           | 12            | 77.7                       | 14.0                                 | 1891               | 31.7         | 1556               | 6.5          | 345        | 364           | 1714                          | 121                | 0.22                   |                             |
| 22988 | 0           | 12            | 77.5                       | 14.5                                 | 1928               | 33.7         | 1539               | 6.4          | 317        | 354           | 1722                          | 119                | 0.21                   |                             |
| 22990 | 20          | 12            | 74.6                       | 14.1                                 | 1939               | 37.3         | 2068               | 7.6          | 554        | 336           | 2002                          | 119                | 0.27                   |                             |
| 22992 | 20          | 12            | 73.4                       | 14.3                                 | 2177               | 36.1         | 1886               | 6.4          | 561        | 332           | 2026                          | 135                | 0.30                   |                             |
| 22996 | 40          | 12            | 86.9                       | 14.0                                 | 1802               | 40.3         | 1931               | 9.1          | 486        | 377           | 1865                          | 99                 | 0.25                   |                             |
| 22997 | 40          | 12            | 83.9                       | 14.5                                 | 1837               | 39.1         | 1766               | 8.6          | 544        | 373           | 1799                          | 101                | 0.31                   |                             |
| 22998 | 60          | 12            | 94.8                       | 13.8                                 | 1419               | 39.2         | 1324               | 9.1          | 445        | 392           | 1369                          | 73                 | 0.34                   |                             |
| 22999 | 60          | 12            | 94.6                       | 14.8                                 | 1756               | 42.2         | 1340               | 9.9          | 520        | 404           | 1534                          | 74                 | 0.39                   |                             |
| 23010 | 0           | 40            | 88.2                       | 14.3                                 | 1881               | 25.3         | 2490               | 6.6          | 924        | 403           | 2162                          | 170                | 0.37                   |                             |
| 23012 | 0           | 40            | 84.2                       | 14.9                                 | 2877               | 32.7         | 2086               | 6.4          | 696        | 435           | 2449                          | 168                | 0.33                   |                             |
| 23015 | 20          | 40            | 87.0                       | 14.0                                 | 2535               | 32.3         | 2701               | 8.0          | 1,155      | 410           | 2615                          | 165                | 0.43                   |                             |
| 23017 | 20          | 40            | 88.2                       | 14.6                                 | 2307               | 31.1         | 2235               | 6.3          | 1,078      | 410           | 2266                          | 162                | 0.48                   |                             |
| 23019 | 40          | 40            | 89.1                       | 14.5                                 | 2833               | 38.0         | 2393               | 8.6          | 968        | 399           | 2602                          | 146                | 0.40                   |                             |
| 23020 | 40          | 40            | 93.8                       | 14.6                                 | 2640               | 39.5         | 2468               | 9.2          | 1,147      | 400           | 2552                          | 134                | 0.46                   |                             |
| 23024 | 60          | 40            | 99.4                       | 14.1                                 | 2342               | 37.6         | 2216               | 9.8          | 1,077      | 431           | 2278                          | 117                | 0.49                   |                             |
| 23025 | 60          | 40            | 92.0                       | 14.5                                 | 2412               | 36.7         | 1868               | 8.6          | 993        | 403           | 2123                          | 119                | 0.53                   |                             |
| 23027 | 40          | 40            | 97.1                       | 14.0                                 | 2148               | 38.0         | 1950               | 9.3          | 810        | 432           | 2043                          | 112                | 0.42                   |                             |
| 23028 | 40          | 40            | 93.4                       | 14.4                                 | 2315               | 37.4         | 2075               | 9.2          | 845        | 416           | 2192                          | 118                | 0.41                   |                             |
| 23032 | 60          | 40            | 104.1                      | 13.8                                 | 2761               | 36.7         | 2453               | 9.3          | 1,325      | 473           | 2602                          | 143                | 0.54                   |                             |
| 23034 | 60          | 40            | 70.6                       | 14.4                                 | 3286               | 38.1         | 3058               | 9.5          | 1,378      | 395           | 3169                          | 169                | 0.45                   |                             |
| 23036 | 40 strat Y* | 40            | 96.8                       | 14.1                                 | 2811               | 38.2         | 2973               | 8.4          | 1,393      | 447           | 2891                          | 159                | 0.47                   |                             |
| 23037 | 40 strat Y* | 40            | 95.9                       | 13.9                                 | 3080               | 37.1         | 3047               | 7.8          | 1,432      | 446           | 3063                          | 177                | 0.47                   |                             |
| 23038 | 40 strat Y* | 40            | 66.0                       | 12.9                                 | 2895               | 37.7         | 2999               | 8.8          | 1,444      | 391           | 2946                          | 163                | 0.48                   |                             |
| 23040 | 40 strat Y* | 40            | 62.4                       | 13.0                                 | 2172               | 37.9         | 2315               | 8.0          | 1,050      | 356           | 2242                          | 129                | 0.45                   |                             |

\*The overall composition of the Yankee side ply is 40% CMF by weight with the Yankee side layer of the headbox issuing substantially 100% CMF.

TABLE 8

| Description        | Basesheet      | CMF        | Softness Panel | Basis Weight lb/3000 ft <sup>2</sup> | Caliper 8 Sheet |                         | MD Tensile g/3 in.   | MD Stretch % | CD Tensile g/3 in. | CD Stretch % |
|--------------------|----------------|------------|----------------|--------------------------------------|-----------------|-------------------------|----------------------|--------------|--------------------|--------------|
|                    |                |            |                |                                      | 8 sht           | lb/3000 ft <sup>2</sup> |                      |              |                    |              |
| 1 P3424.1          | 22989 22988    | 0          | 6.26           | 28.6                                 | 184             | 3,321                   | 29                   | 2,949        | 7.4                |              |
| 2 P3425.1          | 23010 23012    | 0          | 4.88           | 29.6                                 | 204             | 4,057                   | 28                   | 4,547        | 8.3                |              |
| 3 P3426.1          | 23033 23032    | 60         | 4.73           | 27.9                                 | 227             | 5,156                   | 31                   | 4,379        | 9.7                |              |
| 4 P3427.1          | 23034 23032    | 60         | 4.62           | 28.4                                 | 215             | 5,191                   | 30                   | 4,382        | 9.6                |              |
| 5 P3428.1          | 23036 23037    | 40         | 5.37           | 28.0                                 | 221             | 5,007                   | 31                   | 5,082        | 9.1                |              |
| 6 P3429.1          | 23038 23040    | 40         | 5.75           | 25.8                                 | 185             | 4,315                   | 30                   | 4,499        | 8.9                |              |
| 7 P3430.1          | 23024 23025    | 60         | 5.77           | 28.5                                 | 203             | 4,773                   | 34                   | 3,958        | 10.4               |              |
| 8 P3431.1          | 23028 23027    | 40         | 7.29           | 27.7                                 | 205             | 3,791                   | 31                   | 3,624        | 10.2               |              |
| 9 P3432.053        | 23020 23019    | 40         |                | 29.2                                 | 182             | 5,696                   | 35                   | 4,999        | 9.9                |              |
| 10 P3432.083       | 23020 23019    | 40         |                | 29.2                                 | 240             | 4,487                   | 31                   | 4,032        | 9.6                |              |
| 11 P3531.053       | 23028 23027    | 40         |                | 27.8                                 | 183             | 4,413                   | 32                   | 3,970        | 10.0               |              |
| 12 P3531.083       | 23028 23027    | 40         |                | 27.7                                 | 225             | 3,825                   | 31                   | 3,143        | 10.2               |              |
| 13 P3432.1         | 23020 23019    | 40         | 5.14           | 29.2                                 | 205             | 5,377                   | 35                   | 4,672        | 11.1               |              |
| 14 P3433.1         | 22999 22998    | 60         | 8.02           | 28.3                                 | 193             | 3,584                   | 38                   | 3,142        | 12.4               |              |
| 15 P3434.1         | 23015 23017    | 20         | 4.67           | 28.8                                 | 204             | 4,761                   | 32                   | 4,895        | 9.6                |              |
| 16 P3435.1         | 22997 22996    | 40         | 6.75           | 28.7                                 | 186             | 3,579                   | 36                   | 3,535        | 11.0               |              |
| 17 P3436.1         | 22990 22992    | 20         | 6.33           | 29.3                                 | 182             | 3,554                   | 32                   | 3,536        | 8.3                |              |
| GM Tensile g/3 in. | Wet Tens Finch | CD Tensile | SAT Capacity   | SAT Rate g/s <sup>0.5</sup>          | SAT Times       | Break Modulus GM g/%    | Wet Extracted Lint % | Wipe Tops    | Wipe Dry           | Wipe Bottoms |
|                    |                |            |                |                                      |                 |                         |                      |              |                    |              |
| 1                  | 3,128          | 730        | 0.25           | 395                                  | 0.27            | 20                      | 212                  | 0.25         | 19                 | 32           |
| 2                  | 4,293          | 1,380      | 0.30           | 440                                  | 0.33            | 17                      | 283                  | 0.22         | 23                 | 34           |
| 3                  | 4,747          | 2,263      | 0.52           | 438                                  | 0.09            | 105                     | 280                  | 0.09         | 9                  | 9            |
| 4                  | 4,764          | 2,185      | 0.50           | 446                                  | 0.11            | 74                      | 278                  | 0.11         | 12                 | 10           |
| 5                  | 5,042          | 2,262      | 0.45           | 468                                  | 0.12            | 69                      | 300                  | 0.19         | 12                 | 11           |
| 6                  | 4,404          | 1,934      | 0.43           | 418                                  | 0.14            | 42                      | 267                  | 0.17         | 10                 | 9            |
| 7                  | 4,345          | 1,856      | 0.47           | 439                                  | 0.10            | 104                     | 230                  | 0.21         | 11                 | 9            |
| 8                  | 3,705          | 1,494      | 0.41           | 415                                  | 0.10            | 79                      | 210                  | 0.10         | 9                  | 8            |
| 9                  | 5,333          | 1,924      | 0.39           | 409                                  | 0.11            | 79                      | 288                  | 0.28         | 13                 | 13           |

TABLE 8-continued

| Finished Product Data (perforate polymeric belt creped) |       |       |      |     |      |     |     |      |    |    |
|---------------------------------------------------------|-------|-------|------|-----|------|-----|-----|------|----|----|
| 10                                                      | 4,252 | 1,669 | 0.41 | 459 | 0.16 | 42  | 245 | 0.28 | 23 | 11 |
| 11                                                      | 4,184 | 1,677 | 0.42 | 393 | 0.10 | 78  | 235 | 0.09 | 9  | 7  |
| 12                                                      | 3,466 | 1,395 | 0.44 | 451 | 0.12 | 69  | 194 | 0.10 | 9  | 10 |
| 13                                                      | 5,011 | 1,903 | 0.41 | 411 | 0.10 | 79  | 251 | 0.25 | 10 | 13 |
| 14                                                      | 3,356 | 937   | 0.30 | 395 | 0.07 | 133 | 154 | 0.14 | 5  | 5  |
| 15                                                      | 4,825 | 1,745 | 0.36 | 430 | 0.21 | 25  | 276 | 0.21 | 25 | 17 |
| 16                                                      | 3,556 | 1,077 | 0.30 | 391 | 0.09 | 77  | 178 | 0.13 | 9  | 9  |
| 17                                                      | 3,545 | 1,007 | 0.29 | 353 | 0.14 | 37  | 216 | 0.39 | 15 | 18 |

Details as to base-sheet properties and converted two-ply wiper properties appear in Tables 7 and 8. From Table 8, it can be appreciated that the addition of even 20% CMF significantly improves the wipe dry characteristics of the sheets. See lines 15 and 17 in comparison to lines 1 and 2, while improvement in wipe dry starts leveling out with the addition of 40% CMF. Compare line 16 with lines 3, 4 and 7. As is shown in line 14, however, the best overall results for wipe dry and softness were obtained with 60% CMF.

Referring to FIG. 2, it is seen that the two-ply products of the invention exhibit wipe dry and wet tensile that is far superior to that achieved with the conventional towel. As illustrated in FIGS. 10, 11, and 12, it appears that faster wipe dry times may be at least partially attributable to the micropore structure of the sheets formed. In FIG. 10, it can be seen that as CMF is increased, the number of pores less than 5 microns also increases, while the curves for products with 40 or 60% CMF are essentially similar, again, suggesting that only diminishing benefit is obtained beyond 40% CMF. This hypothesis is consistent with that shown in FIG. 10, showing that 20% CMF significantly improves wipe dry, but the effect levels off above 40% CMF. Preferred wiper towel products exhibit a differential pore volume for pores under 5 microns having a diameter of at least about 75 mm<sup>3</sup>/g/micron, more preferably, above about 100 mm<sup>3</sup>/g/micron, still more preferably, above about 150 mm<sup>3</sup>/g/micron for pores under 2.5 microns.

FIG. 11 suggests that there is a correlation between wipe dry and capillary pressure at 10% saturation, both in advancing and receding mode. FIG. 12 shows increasing capillary pressure at 10% saturation as CMF is increased.

FIG. 13 shows wipe dry as a function of CMF and wet strength. Cellulose microfiber (CMF) was varied between 0 and 60%, and Amres® wet strength resin was either 12 lb/ton or 40 lb/ton. Carboxymethylcellulose (CMC) was added at the higher wet strength dosage to balance charge. The non-CMF portion of the furnish was NBSWK refined at a constant net specific horsepower, so that strength changes can be primarily attributed to CMF and resin rather than NBSK refining level. The two curves at roughly constant wet tensile define three planes comprising a 3-D surface on which wipe dry time beneficially decreases as the amount of CMF in the sheet is increased, indicating that wipe dry times of under 10 seconds can be obtained with 40% CMF in the sheet. The surface in FIG. 13 can be described by Equation 1:

$$\text{Wipe Dry} = 22.1 - 0.662 \cdot \text{CMF} + 0.00495 \cdot \text{CMF}^2 + 0.00493 \cdot \text{Wet Tensile} \quad R^2 = 0.99 \quad \text{Equation (1)}$$

FIG. 3 shows the impact of CMF and wet tensile on softness. CMF has a positive impact, while increasing wet tensile strength reduces softness. The surface in FIG. 3 can be described by Equation 2:

$$\text{Softness} = 7.90 + 0.0348 \cdot \text{CMF} - 0.00223 \cdot \text{Wet Tensile} \quad R^2 = 0.99 \quad \text{Equation (2)}$$

FIGS. 2, 14, and 15 illustrate the results of analyses of towels and wipers produced in Example 1, and include retail towel data for comparison. Surprisingly, the inventive product has higher wet tensile at a given softness level than Brawny® towels or Sparkle® towels.

FIGS. 16 and 17 show that wipers with 40% or 60% CMF have very fast wipe dry times, while also having good capacity. FIG. 16 used SAT data, while FIG. 17 used the old water holding capacity test (withdrawn ASTM Standard Method D-4250-92, Standard Method for Water-Holding Capacity of Bibulous Fibrous Products). The general pattern of performance is similar with either test.

FIG. 18 illustrates the counter-intuitive and surprising result that, as CMF is increased, we have found that, even though SAT Rate decreases, wipe dry times decrease.

FIG. 19 illustrates the effect that CMF has upon the wipe dry times at various levels of the wet strength resins Amres® and CMC. It appears that increasing the amount of resin in the outer layers increases the wipe dry times.

FIG. 20 shows wet extracted lint for finished product. CMF typically reduces lint at a variety of levels of CMF and wet strength resins. It can be appreciated that linting generally decreases as the amount of CMF is increased, except that the wet extracted lint generally hovered between 0.20 and 0.25 with the Amres® containing sheets for all levels of CMF.

FIG. 21 shows that any softness benefit from calendering is obtained at a significant cost with respect to lost caliper and absorbency. In one case, a calendered, embossed ply was matched with an unembossed ply for no softness benefit and 12 mil drop in caliper. In another case, a product with two calendered plies had a 0.4 point softness increase, while dropping 35 mils of caliper (see FIG. 21) and 50 gsm SAT. In our experience with softness panels for towel products, a gain of 0.32 points of softness is enough that one product, having a softness panel score 0.32 units greater than another, would be perceived as being noticeably softer, consistently, at the 90% confidence level.

FIG. 22 illustrates the dependence of CD Wet Tensile Strength on both resin addition and CMF. The ratio is higher with CMF at a given resin dose, but the highest ratios are achieved at high CMF and high resin levels.

CMF makes the sheet more difficult to dewater compactively, as the tendency of the sheet to extrude itself out of the pressing nip increases as the CMF content is increased. Oftentimes, this is referred to as sheet crushing. When attempting to dewater a nascent web containing increasing amounts of CMF, the Visconip pressure had to be progressively reduced to prevent sheet crushing at the nip as the level of CMF in the sheet was increased (See FIG. 23). Even though increasing the proportion of CMF in a sheet increases the bulk attainable with a given basis weight (FIG. 24), the reduction in the pressing load that the sheet will sustain results in a wetter sheet going forward, which normally entails much higher expenses for drying energy.

29

FIG. 33 presents SAT Capacity and wipe dry times for both black glass and stainless steel surfaces for the wipers as shown in Example 2.

FIG. 34 is an SEM section (75 $\times$ ) along the machine direction (MD) of perforated polymeric belt creped basesheet 600, showing a domed area corresponding to a belt perforation as well as the densified pileated structure of the sheet. It is seen in FIG. 34 that the domed regions, such as region 640, have a “hollow” or domed structure with inclined and at least partially densified sidewall areas, while surround areas 618, 620 are densified, but less so than transition areas. Sidewall areas 658, 660 are inflected upwardly and inwardly, and are so highly densified as to become consolidated, especially, about the base of the dome. It is believed that these regions contribute to the very high caliper and roll firmness observed. The consolidated sidewall areas form transition areas from the densified fibrous, planar network between the domes to the domed features of the sheet and form distinct regions that may extend completely around and circumscribe the domes at their bases, or may be densified in a horseshoe or bowed shape only around part of the bases of the domes. At least portions of the transition areas are consolidated and also inflected upwardly and inwardly.

30

FIG. 35 is another SEM (120 $\times$ ) along the MD of basesheet 600 showing region 640, as well as consolidated sidewall areas 658 and 660. It is seen in this SEM that the cap 662 is fiber-enriched, of a relatively high basis weight as compared with areas 618, 620, 658, 660. CD fiber orientation bias is also apparent in the sidewalls and dome.

FIG. 36 is an SEM section (120 $\times$ ) along the machine direction (MD) of basesheet 700, in which consolidated sidewall areas 758, 760 are densified and are inflected inwardly and upwardly.

## EXAMPLE 2

### Fabric Creping

Basesheets having the properties set forth in Table 9 were made using fabric creping technology in which the nascent webs were creped from a creping cylinder using a woven creping fabric. These basesheets were converted to finished product towels by embossing one ply with the emboss pattern shown in FIG. 26 (Patches) and glue laminating it to an unembossed ply, as set forth in Tables 9 and 10.

TABLE 9

| FRFC/CMF Basesheet Data, (fabric creped) Basesheet Properties |            |                                                              |             |             |         |        |         |         |         |
|---------------------------------------------------------------|------------|--------------------------------------------------------------|-------------|-------------|---------|--------|---------|---------|---------|
| Cell                                                          | Emboss ply | 2008-1905                                                    | Description | Furnish     | 8 Sheet | Basis  | MD      | CD      | CD Wet  |
|                                                               |            |                                                              |             |             | Caliper | Weight | Tensile | Tensile | Tensile |
| 1                                                             | x          | 14-1                                                         | 19721 229   | 50/50 M/A   | 85.1    | 15.3   | 1754    | 26.4    | 1638    |
|                                                               |            | 15-1                                                         | 19723 239   | 50/50 M/A   | 83.2    | 15.3   | 1695    | 23.3    | 1527    |
| 2                                                             |            | 15 lb/ream Control Average (Calendered)                      |             | 84.1        | 15.3    | 1,724  | 24.9    | 1,582   | 5.5     |
|                                                               | x          | 22-1                                                         | 19731 1008  | 50/50 M/A   | 82.1    | 11.7   | 1745    | 19.8    | 1,454   |
| 3                                                             | x          | 24-1                                                         | 19733 1030  | 50/50 M/A   | 77.1    | 11.6   | 2054    | 20.8    | 1,338   |
|                                                               | x          | 29-1                                                         | 197381140   | 50/50 M/CMF | 79.6    | 11.7   | 1,899   | 20.3    | 1,396   |
| 4                                                             |            | 30-1                                                         | 19739 1154  | 50/50 M/CMF | 95.5    | 12.6   | 2059    | 30.9    | 1,604   |
|                                                               |            | 12 lb/ream Microfiber Average (Uncalendered)                 |             | 94.8        | 12.6    | 1972   | 30.6    | 1,526   | 7.4     |
| 5                                                             | x          | 36-1                                                         | 19755 155   | 50/50 M/CMF | 95.1    | 12.6   | 2,016   | 30.8    | 1,375   |
|                                                               | x          | 37-1                                                         | 19756 205   | 50/50 M/CMF | 110.4   | 14.5   | 2,791   | 33.6    | 2,298   |
| 6                                                             | x          | 37-1                                                         | 19756 205   | 50/50 M/CMF | 114.6   | 13.6   | 2429    | 37.4    | 2160    |
|                                                               | x          | 38-1                                                         | 19757 216   | 50/50 M/CMF | 112.5   | 14.0   | 2,610   | 36.7    | 1,437   |
| 7                                                             | x          | 38-1                                                         | 19757 216   | 50/50 M/CMF | 114.6   | 13.6   | 2,429   | 37.4    | 2160    |
|                                                               | x          | 43-1                                                         | 19762 310   | 50/50 M/CMF | 105.7   | 9.9    | 1,449   | 36.7    | 1,437   |
| 8                                                             |            | 10 lb/ream Microfiber (Uncal, higher FC)                     |             | 105.7       | 9.9     | 1,449  | 36.7    | 1,437   | 8.8     |
|                                                               |            | 10 lb/ream Microfiber (Calendered)                           |             | 59.4        | 9.9     | 1,612  | 27.1    | 1,362   | 8.0     |
| 9                                                             | x          | 41-1                                                         | 19760 248   | 50/50 M/CMF | 94.8    | 10.2   | 1,796   | 31.2    | 1,550   |
|                                                               |            | 42-1                                                         | 19761 300   | 50/50 M/CMF | 93.2    | 10.3   | 1,921   | 29.3    | 1,451   |
| 10                                                            |            | 10 lb/ream Microfiber Average (Uncalendered)                 |             | 940         | 10.2    | 1,859  | 30.2    | 1,501   | 7.9     |
|                                                               |            | M = Northern SW Kraft;<br>A = Araenz <i>Eucahyphus</i> Kraft |             |             |         |        |         |         |         |

TABLE 10

| Base Sheet Assignment and Estimated Finished Product Physical Properties |            |                  |             |                         |                        |                                        |                    |
|--------------------------------------------------------------------------|------------|------------------|-------------|-------------------------|------------------------|----------------------------------------|--------------------|
| cell                                                                     | Emboss Ply | Basesheet Roll # | Sheet Count | Caliper (mils/8 sheets) | Roll Diameter (inches) | CD Wet Tensile ("Finch Cup") (g/3 in.) | Emboss Penetration |
| 1                                                                        | x          | 19721            | 48          | 248 ± 5                 | 5.0 ± 0.1              | 500                                    | 65                 |
|                                                                          |            | 19723            |             |                         |                        |                                        |                    |
| 2                                                                        |            | 19731            | 48          | float                   | float                  | 500                                    |                    |
|                                                                          | x          | 19733            |             |                         |                        |                                        | 65                 |
| 3                                                                        | x          | 19738            | 48          | float                   | float                  | 750                                    | 65                 |
|                                                                          |            | 19739            |             |                         |                        |                                        |                    |
| 4A                                                                       |            | 19755            | 48          | float                   | float                  | 1100                                   |                    |
|                                                                          | x          | 19756            |             |                         |                        |                                        | 65                 |
| 4B                                                                       |            | 19755            | 48          | max                     | >5.0                   | >1100                                  |                    |
|                                                                          | x          | 19756            |             |                         |                        |                                        | 60                 |
| 5A                                                                       | x          | 19756            | 48          | float                   | float                  | 850                                    | 65                 |
|                                                                          |            | 19757            |             |                         |                        |                                        |                    |
| 5B                                                                       | x          | 19756            | 48          | max                     | >5.0                   | >850                                   | 60                 |
|                                                                          |            | 19757            |             |                         |                        |                                        |                    |
| 6A                                                                       |            | 19757            | 48          | float                   | float                  | 700                                    | 65                 |
|                                                                          | x          | 19762            |             |                         |                        |                                        |                    |
| 6B                                                                       |            | 19757            | 48          | float                   | float                  | 700                                    | 60                 |
|                                                                          | x          | 19762            |             |                         |                        |                                        |                    |
| 7A                                                                       | x          | 19760            | 48          | float                   | float                  | 800                                    | 65                 |
|                                                                          |            | 19761            |             |                         |                        |                                        |                    |
| 7B                                                                       | x          | 19760            | 48          | float                   | float                  | 800                                    | 60                 |
|                                                                          |            | 19761            |             |                         |                        |                                        |                    |
| 7C                                                                       | x          | 19760            | 48          | float                   | float                  | 800                                    | 55                 |
|                                                                          |            | 19761            |             |                         |                        |                                        |                    |

When tested for physical properties, the results set forth in Table 11 were obtained. Subsequently, other rolls of basesheet were converted using the emboss design shown in FIG. 25A (Little Circles) in a point to point mode, i.e., registered debosses were formed in the outer surface of each ply with the depths of the debossed regions in each ply being pressed so forcefully against the debossed regions in the other, that the plies are thereby bonded to each other. In some

cases, the contact regions between the plies may be glassined. When Little Circles is used in point to point mode both surfaces show the pattern of FIG. 25A. In cases when a nested mode is used, one surface bears the pattern of FIG. 25A, while the other bears the pattern of FIG. 25B. The physicals of the rolls thereby formed are set forth in Table 11 and the preliminary evaluation of performance is set forth in Table 12.

TABLE 11

| Appendix 1                                                  |                 |       |       |             |       |       |
|-------------------------------------------------------------|-----------------|-------|-------|-------------|-------|-------|
| Properties of Rolls Converted with THVS Emboss in THVS Mode |                 |       |       |             |       |       |
| Cell ID                                                     |                 |       |       |             |       |       |
|                                                             | 1               | 2     | 3     | 4A          | 4B    | 5A    |
| Furnish                                                     |                 |       |       |             |       |       |
|                                                             | 50/50 M/Aracruz |       |       | 50/50 M/CMF |       |       |
| Basis Weight (lb/3000 ft <sup>2</sup> )                     | 29.0            | 23.0  | 24.4  | 27.2        | 26.2  | 22.0  |
| Caliper (mils/8 sheet)                                      | 200             | 180   | 199   | 230         | 214   | 207   |
| MD Tensile (g/3 in.)                                        | 2539            | 2487  | 3599  | 5713        | 6007  | 3638  |
| MD Stretch (%)                                              | 19.2            | 15.6  | 21.1  | 25.1        | 26.3  | 24.1  |
| CD Tensile (g/3 in.)                                        | 2317            | 1974  | 2473  | 3739        | 3738  | 2828  |
| CD Stretch (%)                                              | 5.4             | 5.4   | 7.3   | 6.9         | 7.6   | 8.3   |
| GM Tensile (g/3 in.)                                        | 2423            | 2215  | 2982  | 4620        | 4736  | 3206  |
| CD Wet Tensile-Finch (g/3 in.)                              | 670             | 676   | 1048  | 1749        | 1683  | 1278  |
| CD Tensile Wet/Dry (Unitless)                               | 0.29            | 0.34  | 0.42  | 0.47        | 0.45  | 0.45  |
| SAT Capacity (g/m <sup>2</sup> )                            | 469             | 399   | 447   | 497         | 476   | 460   |
| GM Break Modulus (g/%)                                      | 242.4           | 241.9 | 239.7 | 346.3       | 330.3 | 223.9 |
| GM Modulus (g/% Stretch)                                    | 42.0            | 46.3  | 37.3  | 44.8        | 40.6  | 34.2  |
| Roll Diameter (in)                                          | 4.98            | 4.78  | 4.82  | 5.25        | 4.89  | 4.81  |
| Roll Compress Value (%)                                     | 19.7            | 20.4  | 16.5  | 20.9        | 16.4  | 15.7  |
| Sensory Softness                                            | 8.19            | 6.76  | 6.19  | 4.30        | 4.52  | 5.54  |
| Wet Extracted Lint (%)                                      | 0.069           | 0.050 | 0.063 | 0.076       | 0.080 | 0.062 |
| Wipe Dry Top                                                | 17              | 26    | 14    | 13          | 415   | 15    |
| (Black Glass) (s) Bottom                                    | 16              | 28    | 12    | 15          | 13    | 17    |
|                                                             | Average         | 16    | 27    | 13          | 14    | 16    |
| Wipe Dry Top                                                | 18              | 26    | 14    | 16          | 16    | 22    |
| (Stainless Steel) (s) Bottom                                | 20              | 22    | 15    | 13          | 15    | 14    |
|                                                             | Average         | 20    | 22    | 15          | 13    | 14    |
| Wet Lint (Pigskin)-FQA Fiber Count (Number)                 | 1601            | 808   | 786   | 884         | 814   | 631   |

TABLE 11-continued

| Appendix 1                                                                      |                |       |       |       |       |       |
|---------------------------------------------------------------------------------|----------------|-------|-------|-------|-------|-------|
|                                                                                 | Cell ID        |       |       |       |       |       |
|                                                                                 | 5B             | 6A    | 6B    | 7A    | 7B    | 7C    |
| Furnish                                                                         | 50/50<br>M/CMF |       |       |       |       |       |
| Basis Weight (lb/3000 ft <sup>2</sup> )                                         | 22.1           | 19.5  | 19.4  | 19.5  | 19.6  | 19.6  |
| Caliper (mils/8 sheet)                                                          | 200            | 175   | 165   | 176   | 173   | 169   |
| MD Tensile (g/3 in.)                                                            | 3856           | 2554  | 3051  | 3539  | 3680  | 3971  |
| MD Stretch (%)                                                                  | 24.6           | 20.9  | 21.1  | 21.1  | 21.1  | 21.2  |
| CD Tensile (g/3 in.)                                                            | 3113           | 2332  | 2619  | 2598  | 2702  | 2983  |
| CD Stretch (%)                                                                  | 8.3            | 8.3   | 8.3   | 8.0   | 7.9   | 8.2   |
| GM Tensile (g/3 in.)                                                            | 3464           | 2438  | 2824  | 3031  | 3152  | 3441  |
| CD Wet Tensile-Finch (g/3 in.)                                                  | 1418           | 1095  | 1141  | 1162  | 1263  | 1343  |
| CD Tensile Wet/Dry (Unitless)                                                   | 0.46           | 0.47  | 0.44  | 0.45  | 0.47  | 0.45  |
| SAT Capacity (g/m <sup>2</sup> )                                                | 456            | 408   | 413   | 424   | 411   | 416   |
| GM Break Modulus (g/%)                                                          | 246.4          | 187.2 | 211.4 | 235.2 | 246.0 | 263.1 |
| GM Modulus (g/% Stretch)                                                        | 33.8           | 34.3  | 34.7  | 34.9  | 35.9  | 36.1  |
| Roll Diameter (in)                                                              | 4.77           | 4.55  | 4.35  | 4.67  | 4.63  | 4.34  |
| Roll Compress Value (%)                                                         | 14.5           | 14.6  | 14.3  | 16.5  | 17.2  | 13.5  |
| Sensory Softness                                                                | 5.26           | 7.35  | 6.94  | 5.75  | 5.47  | 5.12  |
| Wet Extracted Lint (%)                                                          | 0.069          | 0.055 | 0.063 | 0.048 | 0.048 | 0.050 |
| Wipe Dry                                                                        | Top            | 14    | 15    | 13    | 14    | 17    |
| (Black Glass) (s)                                                               | Bottom         | 20    | 19    | 18    | 16    | 20    |
|                                                                                 | Average        | 17    | 17    | 15    | 15    | 19    |
| Wipe Dry                                                                        | Top            | 20    | 24    | 21    | 25    | 28    |
| (Stainless Steel) (s)                                                           | Bottom         | 18    | 18    | 19    | 21    | 27    |
|                                                                                 | Average        | 18    | 18    | 19    | 21    | 23    |
| Wet Lint (Pigskin)-FQA Fiber                                                    | 829            | 676   | 577   | 572   | 616   | 594   |
| Count (Number)                                                                  |                |       |       |       |       |       |
| Properties of Rolls Converted with Little Circles Emboss in Point to Point Mode |                |       |       |       |       |       |
|                                                                                 | 4C             | 4D    | 4E    | 7D    | 7E    | 7F    |
| Furnish                                                                         | 50/50 M/CMF    |       |       |       |       |       |
| Basis Weight (lb/3000 ft <sup>2</sup> )                                         | 24.8           | 25.9  | 25.9  | 18.2  | 18.3  | 18.6  |
| Caliper (mils/8 sheet)                                                          | 278            | 234   | 211   | 234   | 224   | 168   |
| MD Tensile (g/3 in.)                                                            | 5188           | 5555  | 6413  | 2749  | 3308  | 4242  |
| MD Stretch (%)                                                                  | 18.0           | 17.9  | 20.3  | 13.2  | 14.3  | 15.7  |
| CD Tensile (g/3 in.)                                                            | 2952           | 3589  | 4203  | 1725  | 2065  | 2934  |
| CD Stretch (%)                                                                  | 10.0           | 9.4   | 8.3   | 10.0  | 9.7   | 8.7   |
| GM Tensile (g/3 in.)                                                            | 3913           | 4460  | 5191  | 2174  | 2612  | 3527  |
| CD Wet Tensile-Finch (g/3 in.)                                                  | 1389           | 1591  | 1865  | 780   | 974   | 1349  |
| CD Tensile Wet/Dry (Unitless)                                                   | 0.47           | 0.44  | 0.44  | 0.45  | 0.47  | 0.46  |
| SAT Capacity (g/m <sup>2</sup> )                                                | 406            | 379   | 405   | 349   | 345   | 342   |
| GM Break Modulus (g/%)                                                          | 289.6          | 341.4 | 401.6 | 188.5 | 224.5 | 300.1 |
| GM Modulus (g/% Stretch)                                                        | 39.1           | 46.0  | 48.8  | 31.2  | 33.8  | 44.2  |
| Roll Diameter (in)                                                              | 5.52           | 5.10  | 4.88  | 5.32  | 5.17  | 4.52  |
| Roll Compress Value (%)                                                         | 14.2           | 13.3  | 15.2  | 16.4  | 16.1  | 15.1  |
| Sensory Softness                                                                | 5.17           | 4.51  | 3.92  | 7.48  | 6.85  | 5.83  |
| Wet Extracted Lint (%)                                                          | 0.057          | 0.082 | 0.075 | 0.050 | 0.052 | 0.056 |
| Wipe Dry                                                                        | Top            | 12    | 12    | 14    | 10    | 16    |
| (Black Glass) (s)                                                               | Bottom         | 17    | 11    | 10    | 17    | 17    |
|                                                                                 | Average        | 14    | 11    | 12    | 14    | 16    |
| Wipe Dry                                                                        | Top            | 15    | 12    | 10    | 17    | 17    |
| (Stainless Steel) (s)                                                           | Bottom         | 12    | 12    | 14    | 10    | 16    |
|                                                                                 | Average        | 12    | 12    | 14    | 10    | 16    |
| Wet Lint (Pigskin)-FQA Fiber                                                    | 561            | 902   | 726   | 679   | 600   | 689   |
| Count (Number)                                                                  |                |       |       |       |       |       |

TABLE 12

| Wipe Dry Data using Wiper Test Method (Single Sheet) (Preliminary Results) |                    |      |      |      |      |      |      |      |      |      |                |      |      |      |      |      |      |      |
|----------------------------------------------------------------------------|--------------------|------|------|------|------|------|------|------|------|------|----------------|------|------|------|------|------|------|------|
| Cell ID                                                                    |                    |      |      |      |      |      |      |      |      |      |                |      |      |      |      |      |      |      |
|                                                                            | 1                  | 2    | 3    | 4A   | 4B   | 5A   | 5B   | 6A   | 6B   | 7A   | 4C             | 4D   | 4E   | 7D   | 7E   | 7F   | 4C   | 4D   |
| Furnish                                                                    | 50/50<br>M/Aracruz |      |      |      |      |      |      |      |      |      | 50/50<br>M/CMF |      |      |      |      |      |      |      |
| Basis Weight (lb/3000 ft <sup>2</sup> )                                    | 29.0               | 23.0 | 24.4 | 27.2 | 26.2 | 22.0 | 22.1 | 19.5 | 19.4 | 19.5 | 24.8           | 25.9 | 25.9 | 18.2 | 18.3 | 18.6 | 24.8 | 25.9 |

TABLE 12-continued

| Wipe Dry Data using Wiper Test Method (Single Sheet) (Preliminary Results) |         |     |     |     |     |     |     |     |     |     |     |     |     |     |     |     |     |     |
|----------------------------------------------------------------------------|---------|-----|-----|-----|-----|-----|-----|-----|-----|-----|-----|-----|-----|-----|-----|-----|-----|-----|
|                                                                            | Cell ID |     |     |     |     |     |     |     |     |     |     |     |     |     |     |     |     |     |
|                                                                            | 1       | 2   | 3   | 4A  | 4B  | 5A  | 5B  | 6A  | 6B  | 7A  | 4C  | 4D  | 4E  | 7D  | 7E  | 7F  | 4C  | 4D  |
| Caliper (mils/8 sheet)                                                     | 200     | 180 | 199 | 230 | 214 | 207 | 200 | 175 | 165 | 176 | 278 | 234 | 211 | 234 | 224 | 168 | 278 | 234 |
| SAT Capacity (g/m <sup>2</sup> )                                           | 469     | 399 | 447 | 497 | 476 | 460 | 456 | 408 | 413 | 424 | 406 | 379 | 405 | 349 | 345 | 342 | 406 | 379 |
| Wipe Dry (Black Glass) (s)                                                 | Top     |     | 92  | 64  | 95  | 133 | 134 | 131 | 123 | 110 | 231 | 115 | 155 | 137 | 165 | 114 | 231 | 115 |
|                                                                            | Bottom  | 59  | 109 | 73  | 113 | 101 | 113 | 133 | 95  | 87  | 222 | 139 | 109 | 129 | 140 | 114 | 222 | 139 |
|                                                                            | Average | 59  | 101 | 68  | 104 | 117 | 123 | 132 | 109 | 99  | 227 | 127 | 132 | 133 | 152 | 114 | 227 | 127 |
| Wipe Dry (Stainless Steel) (s)                                             | Top     | 41  | 64  | 50  | 71  | 59  | 76  | 79  | 69  | 68  | 104 | 69  | 58  | 120 | 78  | 61  | 104 | 69  |
|                                                                            | Bottom  | 43  | 63  | 56  | 49  | 71  | 88  | 81  | 67  | 76  | 78  | 70  | 82  | 134 | 80  | 66  | 78  | 70  |
|                                                                            | Average | 43  | 63  | 56  | 49  | 71  | 88  | 81  | 67  | 76  | 78  | 70  | 82  | 134 | 80  | 66  | 78  | 70  |

By comparing FIGS. 1G, 1J, and 1L, of structures formed by creping from a transfer surface with a perforated polymeric belt, with micrographs of CMF containing structures formed by a variety of other methods, including creping from a transfer surface with a woven fabric, conventional wet pressing, and through-air drying (TAD), it can be appreciated that structures formed by creping from a transfer surface with a perforated polymeric belt exhibit “venation” in some regions in which the CMF fibrils are tightly adhered to an underlying consolidated structure with line contact between the CMF and the underlying consolidated structure. This venation resembles the vein that can be seen in the undersurface of a leaf, and contrasts strongly with the structure formed by the other methods, in which the CMF is part of an open structure more closely resembling ivy growing on a wall than the veins on a leaf. As mentioned previously, without being bound by theory, it is hypothesized that this line surface contact may create micropores that are responsible for the remarkable wipe dry properties of these structures as discussed above. In any event, the superior wipe dry properties of the sheets formed using the perforated polymeric belt and exhibiting venation are undeniable—no matter what the explanation.

FIG. 37 compares the results of Examples 1 and 2 on a normalized basis obtained by dividing the wipe dry time for each cell by the best wipe dry time obtained with a 0% CMF in each of Examples 1 and 2, then plotting these against the CD wet tensile of the wiper in that cell with the fabric creped sheets being indicated by solid symbols, and the samples obtained by creping with a perforated polymeric belt being indicated by hollow symbols in accordance with the legend. It can be appreciated that there is quite a substantial difference between the wipers obtained using the fabric and those using the perforated polymeric belt, particularly, when it is considered that the fabric creped samples indicated by the solid circle contain 50% CMF, while many of the belt creped samples contain far less CMF, the hollow diamonds indicating the presence of 40% CMF and the hollow squares indicating only 20%.

FIG. 38 compares the results of Examples 1 and 2 without normalization of the wipe dry times so that the wipe dry times are compared directly. Again, it can be appreciated that the wipers produced with the perforated polymeric belt are far superior to those produced with a fabric, particularly, when differences in CMF content are considered.

FIG. 39 shows the wipe dry times from Example 1 plotted against the ratio of PAE adhesive to quaternary ammonia salt based release agent in the creping package. It can be appreciated that wipe dry times suffer at low values of this ratio (high levels of quaternary ammonia salt release agent). There-

fore, in those cases when, as is common, the outer surface of the wiper is the Yankee side, care should be exercised to ensure that the level of quaternary ammonium salt retained on the surface of the web is sufficiently low that the wipe dry time is not increased unduly. In the present case, this point is primarily important as being the most likely reason why a few of the wipers with 40% CMF exhibited anomalously high wipe dry times as shown in FIGS. 37 and 38.

While the invention has been described in detail, modifications within the spirit and scope of the invention will be readily apparent to those of skill in the art. In view of the foregoing discussion, relevant knowledge in the art and references including the copending applications discussed above in connection with the Background and Detailed Description, the disclosures of which are all incorporated herein by reference, further description is deemed unnecessary. In addition, it should be understood that aspects of the invention and portions of various embodiments may be combined or interchanged either in whole or in part. Furthermore, those of ordinary skill in the art will appreciate that the foregoing description is by way of example only, and is not intended to limit the invention.

We claim:

1. A method of making multi-ply a wiper/towel product, the method comprising:
  - (a) compactively dewatering a nascent web comprising at least about 10% fibrillated regenerated cellulosic microfibers and having an apparently random distribution of fibers;
  - (b) applying the dewatered web having the apparently random distribution of fibers to a transfer surface;
  - (c) belt-creping the web from the transfer surface utilizing a creping belt, the belt-creping step occurring under pressure in a belt creping nip defined between the transfer surface and the creping belt;
  - (d) drying the web to form a dried web having:
    - (i) a plurality of fiber-enriched hollow domed regions protruding from an upper side of the dried web, the hollow domed regions having a sidewalls of a relatively high local basis weight formed along at least a leading edge thereof;
    - (ii) connecting regions of a relatively lower local basis weight forming a network interconnecting the hollow domed regions of the dried web; and
    - (iii) transition areas with consolidated fibrous regions that transition from the connecting regions into the hollow domed regions, by extending upwardly and inwardly from the connecting regions into the respective sidewalls of the hollow domed regions; and
  - (e) converting said dried web into a multi-ply wiper/towel.

39

2. The method according to claim 1, wherein the nascent web comprises at least about 40% wood pulp derived paper-making fibers.

3. The method according to claim 1, wherein fibrillated regenerated cellulosic microfibers present in the dried web form venation on the surface of the consolidated fibrous regions such that the surface has raised, generally continuous ridges defined thereacross.

4. The method according to claim 1, wherein the consolidated fibrous regions are saddle shaped.

5. The method according to claim 1, wherein the fiber-enriched hollow domed regions exhibit a local basis weight of at least 5% higher than the mean basis weight of a sheet of the product.

6. The method according to claim 1, wherein the fiber-enriched hollow domed regions exhibit a local basis weight of at least 10% higher than the mean basis weight of a sheet of the product.

7. The method according to claim 1, wherein one of at least 20 a portion of the fiber-enriched hollow domed regions and transition areas in the dried web exhibits a cross machine direction (CD) fiber orientation bias.

8. The method according to claim 1, wherein at least a portion of the connecting regions in the dried web exhibits a 25 cross machine direction (CD) fiber orientation bias.

9. The method according to claim 1, wherein at least a portion of the consolidated fibrous regions of the domed region sidewalls in the dried web exhibits a matted structure on both their outer and inner surfaces, and the fibrillated regenerated cellulosic microfibers form venation thereupon, such that the surface has raised, generally continuous ridges defined thereacross.

10. The method according to claim 1, wherein the fibrillated regenerated cellulosic microfibers have a characteristic Canadian Standard Freeness (CSF) value of less than 175 ml.

11. The method according to claim 1, wherein the fibrillated regenerated cellulosic microfibers exhibit a cross machine direction (CD) wet breaking length in the range of about 300 to about 800 m.

12. The method according to claim 11, wherein the fibrillated regenerated cellulosic microfibers exhibit a CD wet breaking length in the range of about 350 to about 800 m.

13. The method according to claim 11, wherein the fibrillated regenerated cellulosic microfibers exhibit a CD wet breaking length in the range of about 400 to about 800 m.

14. The method according to claim 1, wherein the fibrillated regenerated cellulosic microfibers have a number average diameter of less than about 2 microns.

15. The method according to claim 1, wherein the fibrillated regenerated cellulosic microfibers have a number average diameter of from about 0.1 to about 2 microns.

16. The method according to claim 1, wherein the fibrillated regenerated cellulosic microfibers have a fiber count of greater than about 400 million fibers/gram.

17. The method according to claim 1, wherein the fibrillated regenerated cellulosic microfibers have a fiber count of greater than about 50 billion fibers/gram.

18. The method according to claim 1, wherein the fibrillated regenerated cellulosic microfibers have a fiber count 60 greater than about 200 billion fibers/gram.

19. The method according to claim 1, wherein the nascent web comprises from about 10% to about 60% fibrillated cellulosic microfibers.

20. The method according to claim 19, wherein the nascent 65 web comprises at least about 40% wood pulp derived paper-making fibers.

40

21. A method of making multi-ply a wiper/towel product, the method comprising:

(a) compactively dewatering a nascent web comprising at least about 10% fibrillated regenerated cellulosic microfibers and having an apparently random distribution of fibers;

(b) applying the dewatered web having the apparently random distribution of fibers to a transfer surface;

(c) belt-creping the web from the transfer surface utilizing a creping belt, the belt-creping step occurring under pressure in a belt creping nip defined between the transfer surface and the creping belt;

(d) drying the web to form a dried web having:

(i) a plurality of fiber-enriched regions including (A) hollow domed portions having respective sidewalls of a relatively high local basis weight formed along at least a leading edge thereof and (B) piled fiber-enriched portions with a cross machine direction (CD) fiber orientation bias adjacent to the hollow domed portions, the fiber-enriched portions being interconnected with:

(ii) connecting regions of a relatively lower local basis weight,

wherein the hollow domed portions having upwardly projecting densified sidewalls, at least a portion of the upwardly projecting densified sidewalls comprising a densified region that extends inwardly; and

(e) converting said dried web into a multi-ply wiper/towel.

22. The method according to claim 21, wherein the nascent web comprises at least about 40% wood pulp derived paper-making fibers.

23. The method according to claim 21, wherein the fibrillated regenerated cellulosic microfibers exhibit a cross machine direction (CD) wet breaking length in the range of about 300 to about 800 m.

24. The method according to claim 23, wherein the fibrillated regenerated cellulosic microfibers exhibit a CD wet breaking length in the range of about 350 to about 800 m.

25. The method according to claim 23, wherein the fibrillated regenerated cellulosic microfibers exhibit a CD wet breaking length in the range of about 400 to about 800 m.

26. The method according to claim 21, wherein the nascent web comprises from about 10% to about 60% fibrillated regenerated cellulosic microfibers.

27. The method according to claim 26, wherein the nascent web comprises at least about 40% wood pulp derived paper-making fibers.

28. A method of making multi-ply a wiper/towel product, the method comprising:

(a) compactively dewatering a nascent web comprising at least about 10% fibrillated regenerated cellulosic microfibers and having an apparently random distribution of fibers:

(b) applying the dewatered web having the apparently random distribution of fibers to a transfer surface;

(c) belt-creping the web from the transfer surface utilizing a creping belt, the belt-creping step occurring under pressure in a belt creping nip defined between the transfer surface and the creping belt;

(d) drying the web to form a dried web having upper and lower surfaces and comprising:

(i) a plurality of fiber-enriched hollow domed regions protruding from the upper surface of the dried web, the hollow domed regions having respective sidewalls of a relatively high local basis weight formed along at least a leading edge thereof; and

41

- (ii) connecting regions of a relatively lower local basis weight forming a network interconnecting the fiber-enriched hollow domed regions of the dried web; and
- (iii) consolidated groupings of fibers extending upwardly from the connecting regions into the respective sidewalls of the fiber-enriched hollow domed regions,

(e) converting said dried web into a multi-ply wiper/towel.

29. The method according to claim 28, wherein the nascent web comprises at least about 40% wood pulp derived paper-making fibers.

30. The method according to claim 28, wherein the consolidated groupings of fibers extend inwardly and deflect upwardly from the connecting regions into the respective sidewalls of the fiber-enriched hollow domed regions.

31. The method according to claim 28, wherein:

- (i) the fiber-enriched hollow domed regions include an inclined sidewall; and
- (ii) the fibrillated regenerated cellulosic microfibers form venation on the surface of the consolidated groupings of fibers, such that the surface has raised, generally continuous ridges defined thereacross.

32. The method according to claim 28, wherein the fiber-enriched hollow domed regions exhibit a local basis weight of at least 5% higher than the mean basis weight of a sheet of the product.

33. The method according to claim 28, wherein the fiber-enriched hollow domed regions exhibit a local basis weight of at least 10% higher than the mean basis weight of a sheet of the product.

34. The method according to claim 28, wherein the respective sidewalls of the fiber-enriched hollow domed regions comprise regions of consolidated fibers that extend upwardly.

35. The method according to claim 28, wherein consolidated groupings of fibers are saddle shaped and extend upwardly from the connecting regions into the respective sidewalls of the fiber-enriched hollow domed regions.

36. The method according to claim 28, wherein the respective sidewalls of the fiber-enriched hollow domed regions comprise consolidated groupings of fibers that are saddle shaped and extend at least partially around the domed regions.

37. The method according to claim 28, wherein the respective sidewalls extend upwardly and form highly densified consolidated fibrous regions that are saddle shaped about the base of a dome of the domed regions.

38. The method according to claim 28, wherein saddle shaped transition areas with consolidated fibrous regions extend upwardly and inwardly from the connecting regions into the respective sidewalls of the hollow domed regions.

39. The method according to claim 28, wherein the fibrillated regenerated cellulosic microfibers have a fiber count of greater than about 2 billion fibers/gram.

40. The method according to claim 28, wherein the fibrillated regenerated cellulosic microfibers exhibit a cross machine direction (CD) wet breaking length in the range of about 300 to about 800 m.

41. The method according to claim 40, wherein the fibrillated cellulosic microfibers exhibit a CD wet breaking length in the range of about 350 to about 800 m.

42. The method according to claim 40, wherein the fibrillated regenerated cellulosic microfibers exhibit a CD wet breaking length in the range of about 400 to about 800 m.

43. The method according to claim 28, wherein the dried web has transition areas with consolidated fibers that extend upwardly and inwardly from the connecting regions into the respective sidewalls of the hollow domed regions, the transi-

42

tions areas at least partially circumscribe domes of the domed regions at their respective bases.

44. The method according to claim 28, wherein the dried web has transition areas with consolidated fibers that extend upwardly and inwardly from the connecting regions into the sidewalls of the hollow domed regions, the transition areas being densified in a bowed shape around a portion of respective bases of domes of the domed regions.

45. The method according to claim 28, wherein the nascent web comprises from about 10% to about 60% of the fibrillated regenerated cellulosic microfibers.

46. The method according to claim 45, wherein the nascent web comprises at least about 40% wood pulp derived paper-making fibers.

47. A method of making multi-ply a wiper/towel product, the method comprising:

(a) compactively dewatering a nascent web comprising at least about 10% fibrillated regenerated cellulosic microfibers and having an apparently random distribution of fibers;

(b) applying the dewatered web having the apparently random distribution of fibers to a transfer surface;

(c) belt-creping the web from the transfer surface utilizing a creping belt, the belt-creping step occurring under pressure in a belt creping nip defined between the transfer surface and the creping belt;

(d) drying the web to form a dried web comprising:

(i) a plurality of fiber-enriched regions including (A) hollow domed portions having respective sidewalls of a relatively high local basis weight formed along at least a leading edge thereof, the hollow domed portions having upwardly projecting densified sidewalls, at least a portion of each of the upwardly projecting densified sidewalls comprising a densified region that extends inwardly, and (B) piled fiber-enriched portions with a cross machine direction (CD) fiber orientation bias adjacent to the hollow domed portions, the fiber-enriched portions being interconnected with; and

(ii) connecting regions of a relatively lower local basis weight

(e) converting said dried web into a multi-ply wiper/towel.

48. The method according to claim 47, wherein the nascent web comprises at least about 40% wood pulp derived paper-making fibers.

49. The method according to claim 47, wherein the fibrillated regenerated cellulosic microfibers have a Canadian Standard Freeness (CSF) value of less than 175 mL.

50. The method according to claim 47, wherein 40% by weight of the fibrillated regenerated cellulosic microfibers is finer than 14 mesh.

51. The method according to claim 47, wherein at least a portion of each of the upwardly projecting densified sidewalls comprises a densified region that is saddle shaped and extends inwardly.

52. The method according to claim 47, wherein the dried web includes transition areas with consolidated fibrous regions that transition from the connecting regions to the fiber-enriched regions.

53. The method according to claim 47, wherein the fibrillated regenerated cellulosic microfibers have a fiber count of greater than about 400 million fibers/gram.

54. The method according to claim 47, wherein the fibrillated regenerated cellulosic microfibers exhibit a CD wet breaking length in the range of about 300 to about 800 m.

**55.** The method according to claim **54**, wherein the fibrillated regenerated cellulosic microfibers exhibit a CD wet breaking length in the range of about 350 to about 800 m.

**56.** The method according to claim **54**, wherein the fibrillated regenerated cellulosic microfibers exhibit a CD wet breaking length in the range of about 400 to about 800 m.

**57.** The method according to claim **47**, wherein the fibrillated regenerated cellulosic microfibers have a fiber count of greater than about 50 billion fibers/gram.

**58.** The method according to claim **47**, wherein the fibrillated regenerated cellulosic microfibers have a fiber count of greater than about 10 billion fibers/gram.

**59.** The method according to claim **47**, wherein the nascent web comprises from about 10% to about 60% fibrillated regenerated cellulosic microfibers.

**60.** The method according to claim **59**, wherein the nascent web comprises at least about 40% wood pulp derived paper-making fibers.

**61.** A method of making multi-ply a wiper/towel product, the method comprising:

- (a) compactively dewatering a nascent web comprising at least about 10% fibrillated regenerated cellulosic microfibers and having an apparently random distribution of fibers;
- (b) applying the dewatered web having the apparently random distribution of fibers to a transfer surface;
- (c) belt-creping the web from the transfer surface utilizing a creping belt, the belt-creping step occurring under pressure in a belt creping nip defined between the transfer surface and the creping belt;
- (d) drying the web to form a dried web having upper and lower surfaces and comprising:
  - (i) a plurality of fiber-enriched hollow domed regions protruding from the upper surface of the dried web, the hollow domed regions having respective sidewalls of a relatively high local basis weight formed along at least a leading edge thereof; and
  - (ii) connecting regions of a relatively lower local basis weight forming a network interconnecting the fiber-enriched hollow domed regions of the dried web; and
- (e) converting said dried web into a multi-ply wiper/towel.

**62.** The method according to claim **61**, wherein the nascent web comprises at least about 40% wood pulp derived paper-making fibers.

**63.** The method according to claim **61**, wherein the fibrous composition of the web, the geometry of the fibrillated cellulosic microfibers, and the number average count are chosen such that the wiper/towel product exhibits a wipe-dry time of less than about 20 seconds.

**64.** The method according to claim **63**, wherein the wiper/towel product exhibits a wipe-dry time of at most 10 seconds.

**65.** The method according to claim **61**, wherein the fibrillated regenerated cellulosic microfibers exhibit a CD wet breaking length in the range of about 300 to about 800 m.

**66.** The method according to claim **65**, wherein the fibrillated regenerated cellulosic microfibers exhibit a CD wet breaking length in the range of about 350 to about 800 m.

**67.** The method according to claim **65**, wherein the fibrillated regenerated cellulosic microfibers exhibit a CD wet breaking length in the range of about 400 to about 800 m.

**68.** The method according to claim **61**, wherein the fibrous composition of the web, the geometry of the fibrillated regenerated cellulosic microfibers, and the number average count are chosen such that the wiper/towel product exhibits an SAT capacity in the range of about 9.5 to about 11.0 g/g.

**69.** The method according to claim **68**, wherein the sheet exhibits an SAT rate in the range of about 0.05 to about 0.25 g/s<sup>0.5</sup>.

**70.** The method according to claim **61**, wherein consolidated groupings of fibers extend upwardly from the connecting regions into the sidewalls of the fiber-enriched hollow domed regions, and the wiper/towel product exhibits a relative wipe dry time that is less than 50% of the wipe dry time exhibited by a wipe of the same fibrous composition, but without fibrillated regenerated cellulosic microfibers.

**71.** The method according to claim **70**, wherein the product exhibits a relative wipe dry time that is less than about 40% of the wipe dry time exhibited by a wipe of the same fibrous composition, but without fibrillated regenerated cellulosic microfibers.

**72.** The method according to claim **61**, wherein the nascent web comprises from about 10% to about 60% fibrillated regenerated cellulosic microfibers.

**73.** The method according to claim **72**, wherein the nascent web comprises at least about 40% wood pulp derived paper-making fibers.

\* \* \* \* \*